



US007371291B2

(12) **United States Patent**  
**Hayakawa et al.**

(10) **Patent No.:** **US 7,371,291 B2**  
(45) **Date of Patent:** **\*May 13, 2008**

(54) **GRAIN-ORIENTED MAGNETIC STEEL SHEET HAVING NO UNDERCOAT FILM COMPRISING FORSTERITE AS PRIMARY COMPONENT AND HAVING GOOD MAGNETIC CHARACTERISTICS**

(75) Inventors: **Yasuyuki Hayakawa**, Okayama (JP); **Mitsumasa Kurosawa**, Okayama (JP); **Seiji Okabe**, Okayama (JP); **Takeshi Imamura**, Okayama (JP)

(73) Assignee: **JFE Steel Corporation** (JP)

(\*) Notice: Subject to any disclaimer, the term of this patent is extended or adjusted under 35 U.S.C. 154(b) by 303 days.

This patent is subject to a terminal disclaimer.

(21) Appl. No.: **11/145,705**

(22) Filed: **Jun. 6, 2005**

(65) **Prior Publication Data**

US 2005/0224142 A1 Oct. 13, 2005

**Related U.S. Application Data**

(62) Division of application No. 10/312,663, filed as application No. PCT/JP02/00291 on Jan. 17, 2002, now Pat. No. 6,942,740.

(30) **Foreign Application Priority Data**

Jan. 19, 2001 (JP) ..... 2001-011409  
Jan. 19, 2001 (JP) ..... 2001-011410  
Jan. 26, 2001 (JP) ..... 2001-018104  
Jan. 30, 2001 (JP) ..... 2001-021467

(51) **Int. Cl.**

**H01F 1/16** (2006.01)  
**H01F 1/147** (2006.01)

(52) **U.S. Cl.** ..... **148/111; 148/113**

(58) **Field of Classification Search** ..... None  
See application file for complete search history.

(56)

**References Cited**

**U.S. PATENT DOCUMENTS**

5,250,123 A \* 10/1993 Yashiki et al. ..... 148/111  
5,614,034 A \* 3/1997 Suga et al. ..... 148/111  
6,248,185 B1 6/2001 Kondo et al. .....  
6,309,473 B1 \* 10/2001 Hayakawa et al. ..... 148/111  
6,423,157 B2 \* 7/2002 Hayakawa et al. ..... 148/308  
6,811,619 B2 \* 11/2004 Hayakawa et al. ..... 148/111  
RE39,482 E \* 2/2007 Hayakawa et al. ..... 148/111

**FOREIGN PATENT DOCUMENTS**

EP 0 892 072 A1 1/1999  
EP 0 997 540 A1 5/2000  
EP 1 004 680 A1 5/2000

(Continued)

*Primary Examiner*—John P. Sheehan

(74) *Attorney, Agent, or Firm*—DLA Piper US LLP

(57) **ABSTRACT**

A grain oriented electromagnetic steel sheet is free from an undercoating mainly composed of forsterite ( $Mg_2SiO_4$ ), excellent in processability and magnetic properties and useful to production cost, and has a composition containing, by % by mass, 2.0 to 8.0% of Si, wherein secondary recrystallized grains contains fine crystal grains having a grain diameter of 0.15 mm to 0.50 mm at a rate of 2 grains/cm<sup>2</sup> or more. In the process of producing the steel sheet, inhibitors are not utilized, and the fine crystal grains are achieved by high purification and low temperature final annealing.

**17 Claims, 20 Drawing Sheets**



FOREIGN PATENT DOCUMENTS

|    |              |         |    |              |                     |
|----|--------------|---------|----|--------------|---------------------|
| EP | 1 108 794 A1 | 6/2001  | JP | 07-197126    | 8/1995              |
| JP | 60-039123    | 2/1985  | JP | 08-134542    | 5/1996              |
| JP | 63-216945    | 9/1988  | JP | 08-134542 A  | 5/1996              |
| JP | 64-055339    | 3/1989  | JP | 10-17931 A   | 1/1998              |
| JP | 02-057635    | 2/1990  | JP | 10-81915     | 3/1998              |
| JP | 06-49948     | 4/1990  | JP | 2000-087139  | 3/2000              |
| JP | 06-49949     | 4/1990  | JP | 2000-119823  | 4/2000              |
| JP | 07-42556     | 11/1990 | JP | 2000-129356  | 5/2000              |
| JP | 03-111516    | 5/1991  | JP | 2001-32021 A | 2/2001              |
| JP | 04-362132    | 12/1992 | JP | 2002-146491  | 5/2002              |
| JP | 06-17137     | 1/1994  | JP | 2002-217012  | 8/2002              |
| JP | 07-018333    | 1/1994  | WO | WO 98/20179  | 5/1998              |
| JP | 07-076732    | 3/1995  |    |              | * cited by examiner |

## FIG. 1



FIG. 2



FIG. 3



FIG. 4



FIG. 5



FIG. 6



FIG. 7



FIG. 8



FIG. 9



FIG. 10



FIG. 11



→ 1cm ←

MACRO STRUCTURE AFTER FINAL ANNEALING

FIG. 12



FIG. 13



FIG. 14



FIG. 15



FIG. 16



FIG. 17



FIG. 18



FIG. 19



FIG. 20



**GRAIN-ORIENTED MAGNETIC STEEL  
SHEET HAVING NO UNDERCOAT FILM  
COMPRISING FORSTERITE AS PRIMARY  
COMPONENT AND HAVING GOOD  
MAGNETIC CHARACTERISTICS**

**RELATED APPLICATION**

This application is a divisional of application Ser. No. 10/312,663, filed Nov. 27, 2002, now U.S. Pat. No. 6,942,740 which is a §371 of PCT/JP02/00291, filed Jan. 17, 2002, incorporated herein by reference.

**TECHNICAL FIELD**

This disclosure relates to a grain oriented electromagnetic steel sheet suitably used for iron core materials of transformers, motors, electric generators, etc., and a method of producing the steel sheet. The steel sheets can be suitably used for general iron cores, and EI cores particularly used as iron cores of small transformers, and iron core materials of power supply transformers and control elements, which are used at frequencies of 100 to 10000 Hz higher than the commercial frequency, etc.

**BACKGROUND**

Grain oriented electromagnetic steel sheets are widely used as iron cores of transformers, motors, and the like. These materials have crystal orientations highly accumulated in  $\{110\}<001>$  orientation referred to as "Goss orientation", and the properties thereof are mainly evaluated by electromagnetic properties such as magnetic permeability, iron loss, etc.

In the process for producing a grain oriented electromagnetic steel sheet, an undercoating (glass coating) mainly composed of forsterite ( $Mg_2SiO_4$ ) is generally formed on the surface thereof and suitably used as an insulating film and tension applying film. However, this film has the following problems.

In using a grain oriented electromagnetic steel sheet for an iron core of a transformer, a motor, or the like, the steel sheet must be processed into a predetermined shape by punching or shearing. Therefore, the grain oriented electromagnetic steel sheet is required to have the above electromagnetic properties and good processability. Particularly, a small-sized iron core called an EI core used for a power supply adapter, a fluorescent lamp, and the like comprises many laminated steel sheets, and thus punching quality of the electromagnetic steel sheet is an important problem which determines productivity of EI cores in mass production thereof.

The EI core will be described in detail below. FIG. 1 shows an example of the shape of the EI core. The EI core is produced by punching, but an effective processing method producing only a small amount of scrap in punching is used.

As an iron core material for the EI core, both a non-oriented electromagnetic steel sheet and a grain oriented electromagnetic steel sheet are used at present.

The grain oriented electromagnetic steel sheet has good magnetic properties in the rolling direction, but has much interior magnetic properties in the direction perpendicular to the rolling direction. However, in the EI core, a magnetic flux flows at an area ratio of about 20% in the direction perpendicular to the rolling direction, and flows at an area ratio of about 80% in the rolling direction. Therefore, when the grain oriented electromagnetic steel sheet is used as an

ion core material of the EI core, much better properties can be obtained, as compared with the non-oriented electromagnetic steel sheet. Thus, the grain oriented electromagnetic steel sheet is used for many cases in which an iron loss is regarded as important.

As described above, the EI core is produced by punching a steel sheet using a die, but the forsterite undercoating is extremely harder than an organic resin film coated on the non-oriented electromagnetic steel sheet, thereby causing great abrasion of the punching die. Therefore, the die must be early re-polished or exchanged, causing deterioration in the working efficiency of core processing by a user and an increase in cost. Also, the presence of the forsterite undercoating deteriorates a slit property and cutting property.

15 The surface of the grain oriented electromagnetic steel sheet used for this purpose is required to be free from the forsterite undercoating firstly, and many proposals have been made. An example of conceivable methods is a method in which a forsterite undercoating is formed, and then removed by pickling, chemical polishing, electropolishing, or the like. However, this method has a large problem in which the cost is increased, and the surface properties are worsened to deteriorate magnetic properties.

20 Recently, an attempt has been made to control the components of an annealing separator so as not to form a forsterite undercoating or decompose the forsterite undercoating immediately after the forsterite undercoating is formed, producing a grain oriented electromagnetic steel sheet having good processability.

25 For example, Japanese Unexamined Patent Application Publication No. 60-39123 discloses a method of inhibiting the production of a forsterite undercoating by using  $Al_2O_3$  as a main component of an annealing separator. Also, Japanese Unexamined Patent Application Publication No. 6-17137 discloses a method of adding at least one of chlorides, carbonates, nitrates, sulfates and sulfides of Li, K, Na, Ba, Ca, Mg, Zn, Fe, Zr, Sn, Sr, Al, and the like to an annealing separator comprising  $MgO$  as a main component to decompose the formed forsterite undercoating. Furthermore, Japanese Unexamined Patent Application Publication No. 7-18333 discloses a method of removing a  $SiO_2$  undercoating formed in decarburization annealing by using an annealing separator containing 0.2% to 15% of Bi chloride and setting the nitrogen partial pressure of the final annealing atmosphere to 25% or more.

30 These means are capable of producing a grain oriented electromagnetic steel sheet without forming the forsterite undercoating. However, any one of these methods comprises the step of producing the forsterite undercoating or the oxide undercoating composed of  $SiO_2$  as a main component and then decomposing the undercoating, and requires a special releasing agent or auxiliary agent, thereby inevitably complicating the production process and causing the problem of increasing the cost.

35 For example, Japanese Examined Patent Application Publication No. 6-49948 and Japanese Examined Patent Application Publication No. 6-49949 propose a technique for suppressing the formation of a forsterite undercoating by mixing an agent with an annealing separator mainly composed of  $MgO$  and used for final annealing, and Japanese Unexamined Patent Application Publication No. 8-134542 proposes a technique for suppressing the formation of a forsterite undercoating by using an annealing separator 40 mainly composed of silica and alumina for a material containing Mn. However, these methods can remove the adverse effect of the forsterite undercoating, but the problem

of the coarse crystal grains of the grain oriented electromagnetic steel sheet is left unsolved.

Namely, the crystal grains of the grain oriented electromagnetic steel sheet are generally coarsened (usually about 10 to 50 mm) in the process of obtaining the strong Goss texture. Therefore, there is the problem of causing a large change in shape such as shear dropping or the like during punching, as compared with the non-oriented electromagnetic steel sheet generally comprising fine crystal grains of 0.03 to 0.20 mm. On the other hand, a usual method of suppressing the formation of coarse grains deteriorates the magnetic properties such as core loss, etc.

Therefore, means for satisfying both good punching ability and the magnetic properties such as core loss, etc. of the grain oriented electromagnetic steel sheet has not yet been established.

Furthermore, as described above, the grain oriented electromagnetic steel sheet has good magnetic properties in the rolling direction, but poor magnetic properties in the direction perpendicular to the rolling direction. Therefore, in application to the EI core in which a magnetic flux also flows in the direction perpendicular to the rolling direction, it is not said to make sufficient use of the properties of the grain oriented electromagnetic steel sheet.

For this problem, a method of developing a  $(100)<001>$  texture (regular cubic texture) by secondary recrystallization, i.e., a method of producing a so-called two-direction oriented electromagnetic steel sheet, has been investigated from old times.

For example, Japanese Examined Patent Application Publication No. 35-2657 discloses a method comprising performing cold rolling in one direction, performing cold rolling in a direction crossing the one direction to perform cross rolling, and then performing annealing for a short time and annealing at a high temperature of 900 to 1300°C. to obtain a strong cube texture in which regular cubic orientation grains are integrated by secondary recrystallization (using an inhibitor). Japanese Unexamined Patent Application Publication No. 4-362132 discloses a method comprising performing cold rolling with a rolling reduction of 50 to 90% in the direction perpendicular to the hot rolling direction, performing annealing for primary recrystallization, and then performing final annealing for secondary recrystallization and purification to secondarily recrystallize the regular cubic-orientation grains by using AlN.

Although a two-direction oriented electromagnetic steel sheet having good magnetic properties in both the rolling direction and the direction perpendicular to the rolling direction is most useful from the viewpoint of magnetic properties, cross rolling with very low productivity is required for producing the two-direction oriented electromagnetic steel sheet. Therefore, such a two-direction oriented electromagnetic steel sheet has not yet been put into industrial mass production.

Furthermore, in order to apply to the split core of a motor, Japanese Unexamined Patent Application Publication No. 2000-87139 discloses a technique of decreasing inhibitor components to develop the Goss orientation with a low degree of integration, decreasing anisotropy of the magnetic properties of the grain oriented electromagnetic steel sheet. However, this technique deteriorates the degree of integration of the Goss orientation and limits the Si amount to less than 3.0% by mass, and thus in an example, the iron loss  $W_{15/50}$  in the rolling direction is 2.1 W/kg or more, which is, at best, substantially the same as a high-quality non-oriented electromagnetic steel sheet, and is notably worse than the

level of  $W_{15/50} < 1.4$  W/kg of the grain oriented electromagnetic steel sheet. Therefore, this technique does not satisfy the requirements of users.

Apart from the above-described requirements, in some cases, iron core materials are required to exhibit a low iron loss in a high frequency region. Although whether or not this property is affected by the forsterite undercoating has not been known, the inventors found that a steel sheet without the forsterite undercoating developed by the inventors is very suitable for improving the high-frequency iron loss. Therefore, the technical background of this field is described here.

As a method of producing a grain oriented electromagnetic steel sheet having excellent high-frequency iron loss, 15 Japanese Examined Patent Application Publication No. 7-42556 discloses a technique in which a grain oriented electromagnetic steel sheet having a highly developed Goss texture is used as a raw material, cold-rolled with a rolling reduction of 60 to 80% and then subjected to primary 20 recrystallization annealing to obtain a product having a developed Goss texture and a thickness of 0.15 mm or less and comprising fine crystal grains having an average grain diameter of 1 mm or less.

However, this method comprises removing the forsterite 25 undercoating from the grain oriented electromagnetic steel sheet, and performing rolling and recrystallization annealing, and thus this method costs much and is unsuitable for mass production.

Japanese Unexamined Patent Application Publication 30 Nos. 64-5539, 2-57635, 7-76732 and 7-197126 disclose a method of producing a grain oriented electromagnetic steel thin sheet by using surface energy as a driving force without using an inhibitor.

However, there is a problem in which final annealing must 35 be performed at a high temperature under conditions for suppressing the formation of a surface oxide in order to use the surface energy. For example, Japanese Unexamined Patent Application Publication No. 64-55339 discloses that a vacuum, an inert gas, a hydrogen gas, or a mixture of 40 hydrogen gas and nitrogen gas must be used as an atmosphere of final annealing at a temperature of 1180°C. Japanese Unexamined Patent Application Publication No. 2-57635 recommends using an inert gas atmosphere, a hydrogen gas, or a mixed atmosphere of hydrogen gas and inert gas at a temperature of 950 to 1100°C. and further reducing the pressure of the gas. Furthermore, Japanese Unexamined Patent Application Publication No. 7-197126 discloses that final annealing is performed at a temperature of 1000 to 1300°C. in a non-oxidizing atmosphere at an 50 oxygen partial pressure of 0.5 Pa or less or a vacuum.

As described above, in order to obtain good magnetic properties by using the surface energy, an inert gas or hydrogen is used as the atmosphere of final annealing, and a vacuum condition is required as a recommended condition.

55 However, in view of equipment, it is very difficult to set both a high temperature and vacuum, thereby increasing the cost. When the surface energy is utilized, only the  $\{110\}$  plane can be basically selected, and growth of Goss grains in the  $<001>$  orientation coinciding with the rolling direction is not selected.

In the grain oriented electromagnetic steel sheet, the magnetic properties are improved by orienting the easy magnetization axis  $<001>$  in the rolling direction, and thus good magnetic properties are basically not obtained only by 60 selecting the  $\{110\}$  plane.

Therefore, the rolling conditions and annealing conditions for obtaining good magnetic properties by a method using

the surface energy are extremely limited, and thus the magnetic properties become unstable.

As described above, a method of obtaining a good high-frequency iron loss with a high cost efficiency has not yet been found.

As described above, the conventional techniques cannot produce a grain oriented electromagnetic steel sheet having good magnetic properties at low cost, and economically produce a grain oriented electromagnetic steel sheet having good punching quality without forming a forsterite under-coating on the surface.

In consideration of the above situation, it could be advantageous to provide a completely new grain oriented electromagnetic steel sheet excellent in processability and magnetic properties and economically advantageous, and a useful method of producing the same. The application of the steel sheet is not limited, but the steel sheet is ideally used as core materials of small-sized transformers, such as an EI core and the like.

It could also be advantageous to provide a grain oriented electromagnetic steel sheet further satisfying two-direction magnetic properties suitable for EI core materials, and a useful method of producing the steel sheet.

It could further be advantageous to provide a grain oriented electromagnetic steel sheet having highly developed Goss orientation and thus a high magnetic flux density, fine grains appropriately present in secondary recrystallized grains, and excellent iron loss in the high frequency region, and a useful method of producing the steel sheet.

In a process for producing a grain oriented electromagnetic steel sheet, inhibitor elements, for example, MnS, MnSc or AlN, are generally contained in a steel slab used as a starting raw material to selectively grow Goss orientation crystal grains. Therefore, in finish annealing, a so-called "purification annealing process," i.e., annealing at a high temperature of 1200 to 1300° C. in a pure hydrogen stream, is required, and it is thus very difficult to avoid the problems of forming a coating, coarsening the grains and increasing the cost.

On the other hand, as a result of intensive research on the reason for secondary recrystallization of {110} <001> orientation grains, we found that grain boundaries having an orientation difference angle of 20 to 45° in a primary recrystallized structure play an important role, and reported this finding in Acta Material, Vol. 45 (1997), p.1285. This shows that the function of the inhibitor is to produce a "difference between the moving speeds of high-energy grain boundaries and other grain boundaries, and even if the inhibitor is not used, secondary recrystallization is allowed to take place by producing a difference between the moving speeds of the grain boundaries.

On the basis of this finding, we proposed a technique for developing Goss orientation crystal grains by secondary recrystallization of a material not containing the inhibitor component (Japanese Unexamined Patent Application Publication No. 2000-129356).

However, we sought further improvement and conducted intensive research for obtaining a grain oriented electromagnetic steel sheet suitable for small-sized electric apparatuses such as an EI core, in which punching processability is regarded as important.

## SUMMARY

We therefore provide a production method without the formation of an undercoating mainly composed of forsterite is used, a steel raw material containing substantially no

inhibitor component is used, and the ultimate temperature of final annealing is kept down to 1000° C. or lower to leave fine crystal grains, effectively improving an iron loss.

Namely, the construction of a first aspect is as follows:

5 1-1. A grain oriented electromagnetic steel sheet having excellent magnetic properties without an undercoating mainly composed of forsterite ( $Mg_2SiO_4$ ) has a composition containing 1.0 to 8.0% by mass, preferably 2.0 to 8.0 by mass, of Si, wherein secondary recrystallized grains contain 10 fine crystal grains having a grain diameter of 0.15 mm to 0.50 mm at a rate of 2 grains/cm<sup>2</sup> or more.

15 1-2. The grain oriented electromagnetic steel sheet having excellent magnetic properties described above in 1-1 has the composition further containing at least one selected from 0.005 to 1.50% by mass of Ni, 0.01 to 1.50% by mass of Sn, 0.005 to 0.50% by mass of Sb, 0.01 to 1.50% by mass of Cu, 0.005 to 0.50% by mass of P, 0.005 to 0.50% by mass of Mo, and 0.01 to 1.50% by mass of Cr.

20 In the grain oriented electromagnetic steel sheet in the first aspect, the N content is more preferably in the range of 10 to 100 ppm. The grain oriented electromagnetic steel sheet in the first aspect is particularly excellent in the iron loss and punching processability.

25 1-3. A method of producing a grain oriented electromagnetic steel sheet having excellent magnetic properties without an undercoating mainly composed of forsterite comprises hot-rolling a steel slab having a composition containing, by % by mass, 0.08% or less of C, 1.0 to 8.0%, preferably 2.0 to 8.0%, of Si, and 0.005 to 3.0% of Mn, and 30 Al and N decreased to 0.020% or less, preferably 100 ppm or less, and 50 ppm or less, respectively; annealing the hot-rolled sheet according to demand, then cold-rolling the sheet once, or twice or more with intermediate annealing performed therebetween, subsequently recrystallizing and 35 annealing the cold-rolled sheet, and then final annealing the sheet at a temperature of 1000° C. or lower after an annealing separator not containing MgO is coated according to demand.

1-4. In the method of producing the grain oriented electromagnetic steel sheet described above in 1-3, the steel slab further contains, by % by mass, at least one selected from 0.005 to 1.50% of Ni, 0.01 to 1.50% of Sn, 0.005 to 0.50% of Sb, 0.01 to 1.50% of Cu, 0.005 to 0.50% of P, 0.005 to 0.50% of Mo, and 0.01 to 1.50% of Cr.

45 In the production method in the first aspect, recrystallization annealing is preferably performed in a low oxidizing or non-oxidizing atmosphere having a dew point of 40° C. or lower. Also, final annealing is preferably performed in an atmosphere containing nitrogen and/or a low-oxidizing or non-oxidizing atmosphere having a dew point of 40° C. or lower.

50 Also, the slab heating temperature before hot rolling is preferably 1300° C. or lower.

Furthermore, the grain oriented electromagnetic steel sheet obtained is preferably further coated with an insulating coating, and then baked.

55 In the first aspect, by decreasing the C content of the steel slab to 0.006% or less, the decarburization step in annealing can be omitted to permit an attempt to further decrease the cost.

60 Particularly, when the steel slab containing over 100 ppm of Al is used, it is preferable that the steel slab contains, by % by mass, 0.006% or less of C, 2.5 to 4.5% of Si, 0.50% or less of Mn, O suppressed to 50 ppm or less, and the balance substantially composed of Fe and inevitable impurities, the atmosphere of recrystallization annealing has a dew point of 0° C. or lower, the maximum heating tempera-

ture of final annealing is 800° C. or higher, and the rate of heating from 300° C. to 800° C. in final annealing is 5 to 100° C./h.

As a result of intensive research for obtaining magnetic properties suitable for EI core materials based on our above-described technology using a raw material not containing inhibitor components, a second aspect was developed.

We therefore provide a production method without the formation of an undercoating mainly composed of forsterite is used, a steel raw material containing substantially no inhibitor component is used, and the ultimate temperature of final annealing is kept down to 975° C. or lower to leave a predetermined amount of fine crystal grains, effectively improving the iron loss in the direction perpendicular to the rolling direction. The grains are coarsened before final cold rolling to further improve the magnetic flux density and the iron loss in the direction perpendicular to the rolling direction.

Namely, the construction of the second aspect is as follows:

2-1. A grain oriented electromagnetic steel sheet having excellent magnetic properties without an undercoating mainly composed of forsterite ( $Mg_2SiO_4$ ) has a composition containing 1.0 to 8.0% by mass, preferably 2.0 to 8.0 by mass, of Si, wherein secondary recrystallized grains contain fine crystal grains having a grain diameter of 0.15 mm to 0.50 mm at a rate of 2 grains/cm<sup>2</sup> or more, the iron loss ( $W_{L15/50}$ ) in the rolling direction is 1.40 W/kg or less, and the iron loss ( $W_{C15/50}$ ) in the direction perpendicular to the rolling direction is 2.6 times or less as large as that in the rolling direction.

2-2. In the grain oriented electromagnetic steel sheet having excellent magnetic properties described above in 2-1, the magnetic flux density ( $B_{L50}$ ) in the rolling direction is 1.85 T or more, and the magnetic flux density ( $B_{50}$ ) in the direction perpendicular to the rolling direction is 1.70 T or more.

2-3. The grain oriented electromagnetic steel sheet having excellent magnetic properties described above in 2-1 or 2-2 has the composition further containing, by % by weight, at least one selected from 0.005 to 1.50% of Ni, 0.01 to 1.50% of Sn, 0.005 to 0.50% of Sb, 0.01 to 1.50% of Cu, 0.005 to 0.50% of P, 0.005 to 0.50% of Mo, and 0.01 to 1.50% of Cr.

The grain oriented electromagnetic steel sheet in the second aspect has excellent iron losses in the rolling direction and the direction perpendicular to the rolling direction, and excellent punching quality.

2-4. A method of producing a grain oriented electromagnetic steel sheet having excellent magnetic properties without an undercoating mainly composed of forsterite comprises hot-rolling a steel slab having a composition containing, by % by mass, 0.08% or less of C, 1.0 to 8.0%, preferably 2.0 to 8.0%, of Si, 0.005 to 3.0% of Mn, Al decreased to 0.020% or less, preferably 100 ppm or less, and N decreased to 50 ppm or less; annealing the hot-rolled sheet according to demand, cold-rolling the sheet once, or twice or more with intermediate annealing performed therebetween, recrystallizing and annealing the cold-rolled sheet to obtain a grain diameter of 30 to 80  $\mu$ m after annealing, and then final annealing the sheet at a temperature of 975° C. or lower after an annealing separator not containing MgO is coated according to demand.

2-5. A method of producing a grain oriented electromagnetic steel sheet having excellent magnetic properties without an undercoating mainly composed of forsterite comprises hot-rolling a steel slab having a composition

containing, by % by mass, 0.08% or less of C, 1.0 to 8.0%, preferably 2.0 to 8.0%, of Si, 0.005 to 3.0% of Mn, Al decreased to 0.020% or less, preferably 100 ppm or less, and N decreased to 50 ppm or less; annealing the hot-rolled sheet according to demand, cold-rolling the sheet once, or twice or more with intermediate annealing performed therebetween, to obtain a grain diameter of 150  $\mu$ m or more before final cold rolling, recrystallizing and annealing the cold-rolled sheet to a grain diameter of 30 to 80  $\mu$ m after annealing, and then final annealing the sheet at a temperature of 975° C. or lower after an annealing separator not containing MgO is coated according to demand.

2-6. In the method of producing the grain oriented electromagnetic steel sheet described above in 2-4 or 2-5, the steel sheet further contains, by % by mass, at least one selected from 0.005 to 1.50% of Ni, 0.01 to 1.50% of Sn, 0.005 to 0.50% of Sb, 0.01 to 1.50% of Cu, 0.005 to 0.50% of P, 0.005 to 0.50% of Mo, and 0.01 to 1.50% of Cr.

In the production method in the second aspect, the conditions and preferred conditions of the first aspect may be used.

As a result of intensive research finding the probability that magnetic properties suitable for a high-frequency transformer can be obtained based on our technology using a raw material not containing inhibitor components, and optimizing the properties, a third aspect was developed.

We therefore provide a production method without forming an undercoating mainly composed of forsterite is used, a steel raw material containing substantially no inhibitor component is used, and the ultimate temperature of final annealing is kept down to 975° C. or lower to leave fine crystal grains in secondary recrystallized grains, significantly improving the high-frequency iron loss as compared with a conventional grain oriented electromagnetic steel sheet. To secure an area ratio of Goss orientation grains of 50% or more to obtain a good high-frequency iron loss, it is effective to set the grain diameter before final cold rolling to less than 150  $\mu$ m.

Namely, the construction of the third aspect is as follows:

3-1. A grain oriented electromagnetic steel sheet having excellent magnetic properties without an undercoating mainly composed of forsterite ( $Mg_2SiO_4$ ) has a composition containing 1.0 to 8.0% by mass, preferably 2.0 to 8.0 by mass, of Si, wherein the average grain diameter of secondary recrystallized grains in the surface of the steel sheet, which is measured for the grains except fine grains having a grain diameter of 1 mm or less, is 5 mm or more, the secondary recrystallized grains contain fine crystal grains having a grain diameter of 0.15 mm to 0.50 mm at a rate of 2 grains/cm<sup>2</sup> or more and fine crystal grains having a grain diameter of 0.15 mm to 1.00 mm at a rate of 10 grains/cm<sup>2</sup> or more, and the area ratio of crystal grains with an orientation difference of 20° or less from the {110}<001> orientation is 50% or more.

3-2. The grain oriented electromagnetic steel sheet having excellent magnetic properties described above in 3-1 has the composition further containing, by % by mass, at least one selected from 0.005 to 1.50% of Ni, 0.01 to 1.50% of Sn, 0.005 to 0.50% of Sb, 0.01 to 1.50% of Cu, 0.005 to 0.50% of P, 0.005 to 0.50% of Mo, and 0.01 to 1.50% of Cr.

The grain oriented electromagnetic steel sheet in the third aspect has the property of a low high-frequency iron loss.

3-3. A method of producing a grain oriented electromagnetic steel sheet having excellent magnetic properties without an undercoating mainly composed of forsterite comprises hot-rolling a steel slab having a composition containing, by % by mass, 0.08% or less of C, 1.0 to 8.0%,

preferably 2.0 to 8.0%, of Si, 0.005 to 3.0% of Mn, and Al decreased to 0.020% or less, preferably 100 ppm or less, and N decreased to 50 ppm or less, annealing the hot-rolled sheet according to demand, cold-rolling the sheet once, or twice or more with intermediate annealing performed therebetween, to obtain a grain diameter of less than 150  $\mu\text{m}$  before final cold rolling, recrystallizing and annealing the cold-rolled sheet to obtain a grain diameter of 30 to 80  $\mu\text{m}$  after annealing, and then final annealing the sheet at a temperature of 975° C. or lower after an annealing separator not containing MgO is coated according to demand.

In the third aspect, the formation of the forsterite under-coating in final annealing is suppressed to obtain a smooth surface, which is suitable for high-frequency magnetic properties.

3-4. In the method of producing the grain oriented electromagnetic steel sheet described above in 3-3, the steel slab further contains, by % by mass, at least one selected from 0.005 to 1.50% of Ni, 0.01 to 1.50% of Sn, 0.005 to 0.50% of Sb, 0.01 to 1.50% of Cu, 0.005 to 0.50% of P, 0.005 to 0.50% of Mo, and 0.01 to 1.50% of Cr.

In the third aspect, the conditions and preferred conditions in the first or second aspect may be used.

#### BRIEF DESCRIPTION OF THE DRAWINGS

FIG. 1 is a drawing showing the shape of an EI core typical as a small-sized transformer.

FIG. 2 is a graph showing the relationship between the ultimate temperature and atmosphere of final annealing and the magnetic property in the rolling direction of a grain oriented electromagnetic steel sheet.

FIG. 3 is a photograph showing the crystal structure of a test material of the electromagnetic steel sheet shown in FIG. 2 after final annealing.

FIG. 4 is a graph showing the relationship between the ultimate temperature of final annealing and the existence rate of fine grains of the test material shown in FIG. 2.

FIG. 5 is a graph showing the relationship between the existence rate of fine grains and the EI core iron loss of the test material shown in FIG. 2.

FIG. 6 is a graph showing the relationship between the N content of steel and the number of times of punching of the test material shown in FIG. 2.

FIG. 7 is a drawing showing the existence frequencies of grain boundaries with an orientation difference angle of 20 to 45° in a primary recrystallized structure of a grain oriented electromagnetic steel sheet.

FIG. 8 is a graph showing the relationship between the ultimate temperature of final annealing, the presence of an annealing separator and the iron loss in each of the rolling direction and the direction perpendicular to the rolling direction of a grain oriented electromagnetic steel sheet.

FIG. 9 is a graph showing the relationship between the ultimate temperature of final annealing and the ratio of the iron loss in the direction perpendicular to the rolling direction to the iron loss in the rolling direction of the experimental material shown in FIG. 8.

FIG. 10 is a graph showing comparison of changes in the iron loss in each of the rolling direction and the direction perpendicular to the rolling direction with the ultimate temperature of final annealing between before and after removal of a surface coating of each of the grain oriented electromagnetic steel sheet (the experimental material shown in FIG. 8).

FIG. 11 is a photograph showing the crystal structure of the grain oriented electromagnetic steel sheet (the experimental material shown in FIG. 8) after being maintained at 875° C.

5 FIG. 12 is a graph showing the relationship between the existence rate of fine grains and the ratio of the iron loss in the direction perpendicular to the rolling direction to the iron loss in the rolling direction of the experimental material shown in FIG. 8.

10 FIG. 13 is a graph showing the relationship between the grain diameter before final cold rolling and the magnetic flux densities in the rolling direction and the direction perpendicular to the rolling direction of a grain oriented electromagnetic steel sheet.

15 FIG. 14 is a graph showing the relationship between the grain diameter before final cold rolling and the iron losses in the rolling direction and the direction perpendicular to the rolling direction of the experimental material shown in FIG. 13.

20 FIG. 15 is a graph showing the relationship between the ultimate temperature of final annealing, the presence of an annealing separator and the high-frequency iron loss ( $W_{10/1000}$ ) of a grain oriented electromagnetic steel sheet.

FIG. 16 is a graph showing changes in the iron loss before and after removal of a surface oxide coating of each of the experimental materials shown in FIG. 15.

25 FIG. 17 is a graph showing the photofinishing structure of a grain oriented electromagnetic steel sheet (the experimental material shown in FIG. 15) after final annealing.

30 FIG. 18 is a graph showing the relationship between the number of fine grains in the secondary recrystallized grains and the high-frequency iron loss ( $W_{10/1000}$ ) of the experimental material shown in FIG. 15.

35 FIG. 19 is a graph showing the relationship between the high-frequency iron loss ( $W_{10/1000}$ ) and the area ratio of Goss orientation grains of a grain oriented electromagnetic steel sheet.

40 FIG. 20 is a graph showing the relationship between the grain diameter before final cold rolling and the area ratio of Goss orientation grains of the experimental material shown in FIG. 19.

#### DETAILED DESCRIPTION

##### (First Aspect—Operation)

A first aspect is described. Experiment resulting in the success of the first aspect is first described (Experiment 1).

45 A steel slab having a composition free from inhibitor components and containing, by % by mass, 0.0020% of C, 3.5% of Si, 0.04% of Mn, Al and N decreased to 20 ppm and 50 ppm, respectively, and other components decreased to 30 ppm or less was produced by continuous casting. Then, the steel slab was heated to 1150° C., and then hot-rolled to form a hot-rolled sheet of 3.0 mm in thickness. The hot-rolled sheet was soaked at 850° C. for 1 minute in a nitrogen atmosphere, and then rapidly cooled.

55 Then, after a final thickness of 0.35 mm was obtained by cold rolling, recrystallization annealing was carried out by soaking at 930° C. for 20 seconds in two types of atmospheres including an atmosphere containing 50 vol % of hydrogen and 50 vol % of nitrogen and having a dew point of -30° C., and an atmosphere containing 50 vol % of hydrogen and 50 vol % of nitrogen and having a dew point of 50° C.

60 Then, final annealing was performed. In the final annealing, the temperature was increased from room temperature

## 11

to 875° C. at a rate of 50° C./h in a nitrogen atmosphere having a dew point of -20° C., kept for 50 hours, and then further increased to various temperatures at a rate of 20° C./h in the atmosphere changed to a hydrogen atmosphere.

After final annealing, an organic coating (thickness: 1 µm) comprising aluminum bichromate, an acrylic resin emulsion and boric acid was coated.

By using the thus-obtained product sheet (Al reduced to 10 ppm, and other components being the same as or reduced to lower than the levels of the slab components except N), an EI core was formed, and its iron loss ( $W_{15/50}$ ) was measured. For a comparison, an EI core formed by using a commercial grain oriented electromagnetic steel sheet having the same thickness was measured by the same method.

FIG. 2 shows the results of measurement of the relationship between the ultimate temperature of final annealing and the magnetic property. Although the ultimate temperature of final annealing of the commercial grain oriented electromagnetic steel sheet is not known, the commercial grain oriented electromagnetic steel sheet is also shown in the graph for comparison.

This figure indicates that in recrystallization annealing in a dry atmosphere with a dew point of -30° C., a good iron loss is obtained in the range of ultimate temperatures of final annealing of 875 to 950° C., while the iron loss deteriorates at an ultimate temperature of over 1000° C. However, even when the iron loss deteriorates, the iron loss is better than that of the commercial grain oriented electromagnetic steel sheet.

On the other hand, in recrystallization annealing in a wet atmosphere with a dew point of 50° C., the iron loss is worse than that in the dry atmosphere, and only an iron loss close to that of the commercial grain oriented electromagnetic steel sheet can be obtained.

Next, in order to make clear the reason why the good iron loss was obtained in recrystallization annealing in a dry atmosphere, the crystal structure was examined.

FIG. 3 shows the crystal structure after final annealing.

FIG. 3 indicates that fine crystal grains having a grain diameter of about 0.15 to 0.50 mm are scattered in secondary recrystallized coarse grains of as large as several cm. As a result of measurement of a sectional structure, it was found that the fine grains pass through the sheet in the thickness direction.

It is thus found that the existence rate of fine crystal grains (passing through the sheet in the thickness direction unless otherwise stated) having a grain diameter of 0.15 to 0.50 mm and the iron loss of the EI core have a strong correlation therebetween.

FIG. 4 shows the results of measurement of the relationship between the ultimate temperature of final annealing and the existence rate of fine grains. The existence rate of fine grains was determined by measuring the number of fine crystal grains of 0.15 to 0.50 mm in diameter (corresponding to the diameter of a circle) within a 3-cm square region of the surface of the steel sheet.

FIG. 4 indicates that the number of fine grains decreases as the ultimate temperature increases. Namely, at an ultimate temperature of final annealing of 1000° C. or lower, the rate of the fine crystal grains is 2 grains/cm<sup>2</sup> or more, while at an ultimate temperature of 950° C. or lower, the rate is 50 grains/cm<sup>2</sup> or more.

FIG. 5 shows the result of measurement of the relationship between the existence rate of fine grains and the EI core iron loss.

## 12

As shown in FIG. 5, it is made clear that with a rate of fine crystal grains of 2 grains/cm<sup>2</sup> or more, preferably 50 grains/cm<sup>2</sup> or more, a good iron loss is obtained.

Next, in order to evaluate punching quality, continuous punching into a 17-mm square (material: SKD-11) was carried out by using a 25-ton press and commercial punching oil under conditions of a punching rate of 350 strokes/min and a clearance of 6% of thickness until the burr height reached 50 µm.

Table 1 shows the results of measurement of the relationship between the ultimate temperature of final annealing and the number of times of punching.

TABLE 1

| Ultimate temperature (° C.) | Material annealed in dry atmosphere        |                             | Material annealed in wet atmosphere        |                             |
|-----------------------------|--------------------------------------------|-----------------------------|--------------------------------------------|-----------------------------|
|                             | Number of times of punching (10,000 times) | Ultimate temperature (° C.) | Number of times of punching (10,000 times) | Ultimate temperature (° C.) |
| 875                         | >300                                       | 875                         | 100                                        |                             |
| 900                         | >300                                       | 900                         | 90                                         |                             |
| 925                         | >300                                       | 925                         | 80                                         |                             |
| 950                         | 250                                        | 950                         | 50                                         |                             |
| 975                         | 230                                        | 975                         | 30                                         |                             |
| 1000                        | 200                                        | 1000                        | 20                                         |                             |
| 1025                        | 120                                        | 1025                        | 20                                         |                             |
| 1050                        | 100                                        | 1050                        | 20                                         |                             |

Comparative Example (Grain oriented electromagnetic steel sheet) Number of times of punching: 5,000 times

Table 1 indicates that in the case of recrystallization annealing in a dry atmosphere, the punching quality is best, and in the case of recrystallization in a wet atmosphere, the punching quality is worse, and particularly, with the commercial grain oriented electromagnetic steel sheet having the forsterite undercoating, the punching quality significantly deteriorates.

It is also found that in the case of recrystallization annealing in a dry atmosphere, the number of times of punching is good at an ultimate temperature of 1000° C. or lower, and the punching quality is liable to deteriorate as the ultimate temperature increases.

The commercial grain oriented electromagnetic steel sheet has an undercoating mainly composed of forsterite, and forms an internal oxide layer mainly composed of silica by recrystallization annealing in a wet atmosphere, thereby deteriorating the punching quality. However, even in recrystallization annealing in a dry atmosphere, dependency of the number of times of punching on the ultimate temperature was observed.

Therefore, as a result of investigation for making clear the reason for this, it was found that the nitrogen content of steel after final annealing also affects the punching quality.

As a result of examination, it was found that the nitrogen content of steel increases during retention at 875° C., and decreases due to denitridation as the temperature increases to 950° C. or higher.

FIG. 6 shows the relationship between the N content of steel and the number of times of punching. It is notable as shown in FIG. 6 that with an N content of steel of 10 ppm or more, the punching quality is significantly improved.

As described above, the iron loss can be effectively improved by eliminating the surface oxides such as the undercoating, the internal oxide layer, and the like by recrystallization annealing in a dry atmosphere, and by keeping down the ultimate temperature of final annealing to

1000° C. or lower, leaving fine crystal grains. Also, without the undercoating (glass coating) mainly composed of forsterite ( $Mg_2SiO_4$ ), the punching quality can be significantly improved by adding 10 ppm or more of N to steel.

Recrystallization annealing is performed in a low oxidizing or non-oxidizing atmosphere having a dew point of 40° C. or lower to remove the surface oxides such as the forsterite undercoating, the undercoating, and the like, and the ultimate temperature of final annealing is kept down to 1000° C. or lower to leave fine crystal grains. Although the reason why this operation contributes to a decrease in the iron loss is not always made clear, we think the reason as follows.

First, when recrystallization annealing is performed in a low oxidizing or non-oxidizing atmosphere to prevent the formation of the surface oxides, possibly, a magnetically smooth surface is maintained, and a magnetic wall readily moves to decrease a hysteresis loss. Furthermore, the presence of fine crystal grains in secondary recrystallized gains possibly causes subdivision of magnetic domains to decrease an eddy current loss. The conventional technique using the inhibitor can achieve a low iron loss only when the inhibitor components (S, Se, N and the like) are purified by annealing at a high temperature of about 1000° C. or higher, but the method not using the inhibitor can achieve a low iron loss after the completion of secondary recrystallization even when purification is not performed. Therefore, the method of keeping down the ultimate temperature of final annealing leaving fine grains is considered effective.

The conceivable reason why secondary recrystallization is developed in steel not containing the inhibitor components is the following.

As a result of intensive research on the reason for secondary recrystallization of Goss orientation grains, we found that a grain boundary having an orientation difference angle of 20 to 45° in the primary recrystallized structure plays an important role, and reported this finding in *Acta Materialia*, Vol. 45 (1997), p. 1285.

The primary recrystallized structure of the grain oriented electromagnetic steel sheet immediately before the secondary recrystallization was analyzed to examine the ratio (%) of grain boundaries having an orientation difference angle of 20 to 45° to the total grain boundaries around crystal grains having various crystal orientations. The results are shown in FIG. 7. In FIG. 7, the crystal orientation space is indicated by using a section of  $\Phi_2=45^\circ$  of the Eulerian angles ( $\Phi_L$ ,  $\Phi$ ,  $\Phi_2$ ), and main orientations such as the Goss orientation and the like are schematically shown.

FIG. 7 shows the existence frequencies of grain boundaries with orientation difference angles of 20 to 45° in the primary recrystallized structure of the grain oriented electromagnetic steel sheet, the Goss orientation having a highest rate. According to the experimental data of C. G. Dunn et al. (AIME Transaction, Vol. 188 (1949), P. 368), the grain boundaries having an orientation difference angle of 20 to 45° are high-energy grain boundaries. The high-energy grain boundaries have a large free space in the boundaries and a disordered structure. Diffusion along grain boundaries is a process in which atoms move through the grain boundaries, and thus the high-energy grain boundaries having a large free space have a high diffusion rate.

It is known that secondary recrystallization is developed accompanying growth and coarsening due to diffusion control by the precipitates called the inhibitor. Coarsening of the precipitates on the high-energy grain boundaries preferentially proceeds during final annealing, and thus pinning of the grain boundaries of Goss orientation is preferentially

removed to start movement of the grain boundaries, thereby possibly growing Goss orientation grains.

As a result of further progress of the above research, we found that the fundamental factor of preferential growth of the Goss orientation grains in secondary recrystallization is the distribution state of the high-energy grain boundaries in the primary recrystallized structure, and the function of the inhibitor is to produce a difference between the moving velocities of the grain boundaries of the Goss orientation grains, which are high-energy grain boundaries, and other grain boundaries. Namely, since coarsening of the inhibitor on the high-energy grain boundaries preferentially proceeds in secondary recrystallization annealing, pinning by the inhibitor on the high-energy grain boundaries is preferentially removed to start movement of the grain boundaries.

According to this theory, therefore, if the difference between the moving velocities of the grain boundaries can be produced, secondary recrystallization in the Goss orientation can be made without using the inhibitor.

Since the impurity elements present in steel are easily segregated on the grain boundaries, particularly the high-energy grain boundaries, there is possibly no difference between the moving velocities of the high-energy grain boundaries and other grain boundaries when steel contains large amounts of impurity elements.

Therefore, by highly purifying a raw material to remove the influence of the impurity elements, the original difference between the moving velocities depending upon the structure of the high-energy grain boundaries is elicited to permit secondary recrystallization in the Goss orientation.

Furthermore, the reason why the punching quality is further significantly improved by controlling the N content of steel to 10 ppm or more is possibly that a small amount of solute nitrogen as interstitial dissolved element has an influence. Also, the presence of fine crystal grains themselves scattered in the secondary recrystallized grains, which are possibly increased by remaining N, possibly contributes to improvement in the punching quality.

In the conventional technique, it has been said that the inhibitor must be finely diffused in steel to develop secondary recrystallized grains, and thus a steel slab must be heated to a high temperature of above 1300° C. to 1400° C. before hot rolling. To prevent coarsening of crystal grains by high-temperature heating to form a homogeneous structure, steel conventionally contains 0.04% to 0.08% of C. However, based on our idea that secondary recrystallization can be made with a highly-purified raw material, the inhibitor need not be diffused in steel. Therefore, the heating temperature of the slab can be decreased.

Furthermore, it is unnecessary to add C to the starting raw material, and progress decarburization in primary recrystallization annealing, and thus primary recrystallization annealing can be performed in a dry atmosphere to suppress the formation of  $SiO_2$  in the surface layer of the steel sheet. As a result, the formation of the forsterite undercoating can be further suppressed.

When the steel slab contains over 100 ppm of Al, as a means for securing fine crystal grains having a grain diameter of 0.15 to 0.50 mm at a ratio of 2 grains/cm<sup>2</sup> or more to obtain a good iron loss, it is preferably to set (1) the rate of heating from 300° C. to 800° C. to 5 to 100° C./h, and (2) the maximum heating temperature to 800° C. or higher.

The reason why the behavior of secondary recrystallization depends upon the heating rate of secondary recrystallization annealing when steel contains a large amount of Al is not made clear. However, it is presumed that with a heating rate of as low as less than 5° C./h, small amounts of

impurity elements are concentrated and precipitated before grain growth to partially suppress grain growth in some cases. While with a heating rate of as high as over 100° C./h, there is substantially no time difference between the temperature of movement of high-energy grain boundaries and the temperature of movement of low-energy grain boundaries, and thus all grain boundaries move at substantially the same time to exhibit the behavior of normal grain growth in some cases.

When the slab contains over 100 ppm (0.020% or less) of Al, the above methods (1) and (2) for improving the iron loss are effective for the case in which the slab composition satisfies 0.0060% or less of C, 2.5 to 4.5% of Si, 0.50% or less of Mn, and 50 ppm or less of O (all in % by mass) besides Al and N, and the balance is preferably composed of Fe and inevitable impurities. The Al content is more preferably less than 150 ppm. Furthermore, the dew point of final annealing is preferably 0° C. or less.

(First aspect—Limitation and Preferred Range)

A description will now be made of the reasons for limiting the features of the first aspect.

First, the grain oriented electromagnetic steel sheet of the first aspect must contain as a component, by % by mass, 1.0 to 8.0% of, preferably 2.0 to 8.0% of, Si.

This is because with a Si content of less than 1.0%, the sufficient effect of improving the iron loss cannot be obtained, while with a Si content of over 8.0%, processability deteriorates. In order to obtain the excellent effect of improving the iron loss, the Si content is preferably in the range of 2.0% to 8.0%.

In order to secure processability, it is preferable to add 10 ppm or more of N. However, in order to avoid deterioration of the iron loss, the amount of N added is preferably 100 ppm or less.

To decrease the iron loss of the steel sheet, secondary recrystallized grains must contain fine crystal grains having a grain diameter of 0.15 mm to 0.50 mm at a rate of 2 grains/cm<sup>2</sup> or more, preferably 50 grains/cm<sup>2</sup> or more.

When the fine grains have a grain diameter of less than 0.15 mm or over 0.50 mm, the effect of subdividing magnetic domains is small, and thus do not contribute to a decrease in the iron loss. Therefore, consideration is given to the existence rate of the fine crystal grains having a grain diameter in the range of 0.15 mm to 0.50 mm, but with the fine crystal grains with an existence rate of less than 2 grains/cm<sup>2</sup>, the effect of subdividing magnetic domains is decreased to fail to expect a sufficient improvement in the iron loss. Although the upper limit of the existence rate of the fine crystal grains is not limited, the upper limit is preferably about 1000 grains/cm<sup>2</sup> because an excessively high rate decreases the magnetic flux density.

In order to secure good punching quality, a major premise is that the undercoating mainly composed of forsterite ( $Mg_2SiO_4$ ) is not formed on the surface of the steel sheet.

Next, the reasons for limiting the components of the raw material slab for producing the electromagnetic steel sheet are described. In the composition below, “%” is “% by mass”.

C: 0.08% or less

With the raw material having a C amount of over 0.08%, C cannot be easily decreased to about 50 to 60 ppm or less, which causes no magnetic aging, even by decarburization annealing, and thus the C amount must be limited to 0.08% or less. Particularly, in the stage of the raw material, the C amount is preferably decreased to 60 ppm (0.006%) or less in order to obtain a product having a smooth surface by

intermediate annealing or recrystallization annealing in a dry atmosphere without decarburization.

Namely, by omitting decarburization, the opportunity of forming a  $SiO_2$  coating in the surface layer of the steel sheet 5 can be removed to prevent the punching quality of a product from deteriorating due to the  $SiO_2$  coating, and further by a hard coating from being formed by reaction between the  $SiO_2$  coating and an annealing separator in secondary recrystallization annealing. Also, the possibility of formation of coarse grains during decarburization can be avoided.

Mn: 0.005 to 3.0%

Mn is a necessary element for improving hot processability, but an adding amount of less than 0.005% has a low effect, while an adding amount of over 3.0% decreases the 15 magnetic flux density. Therefore, the Mn amount is 0.005 to 3.0%.

In view of the magnetic properties and the alloy cost, the Mn amount is preferably 0.50% or less.

As described above for the electromagnetic steel sheet as 20 a product sheet, the Si amount is 1.0 to 8.0%, preferably 2.0 to 8.0%.

From the viewpoint of avoiding deterioration in the magnetic properties due to  $\gamma$ -transformation in annealing or the like in a high temperature region, the Si content is 25 preferably 2.5% or more. Also, from the viewpoint of securing the saturation magnetic flux density, the Si content is preferably 4.5% or less.

Al: 0.020% or less (preferably 100 ppm or less), N: 50 ppm or less

In order to sufficiently develop secondary recrystallization, the Al content must be decreased to 0.020% or less, preferably less than 150 ppm, more preferably 100 ppm or less, and the N content must be decreased to 50 ppm or less, preferably 30 ppm or less.

Furthermore, it is advantageous to minimize the inhibitor forming elements S, Se and the like (the elements generally contained in the grain oriented electromagnetic steel sheet in order to form the inhibitor) to 50 ppm or less, preferably 30 ppm or less.

40 In order to prevent deterioration in the iron loss and secure processability, it is advantageous to decrease the nitride forming elements, Ti, Nb, Ta, V and the like, to 50 ppm or less each. Since B is both a nitride forming element and an inhibitor forming element, and has an influence even when the content is small, the B content is preferably 10 ppm or less.

Also, O may be a harmful element which inhibits the 50 generation of secondary recrystallized grains, and may be left in matrix to cause deterioration in the magnetic properties, and thus the O content is 50 ppm or less, and preferably 30 ppm or less.

Although the essential components and the inhibited components are described above, the other elements described below can also be appropriately added.

55 Namely, in order to improve the structure of a hot-rolled sheet to improve the magnetic properties, Ni can be added. However, with an adding amount of less than 0.005%, the magnetic properties such as an iron loss and the like are less improved, while with an adding amount of over 1.50%, secondary recrystallization is destabilized to deteriorate the magnetic properties such as an iron loss and the like. Therefore, the amount of Ni added is preferably 0.005 to 1.50%, and more preferably 0.01% or more.

Furthermore, in order to improve the iron loss, 0.01 to 60 1.50% of Sn, 0.005 to 0.50% of Sb, 0.01 to 1.50% of Cu, 0.005 to 0.50% of P, 0.005 to 0.50% of Mo and 0.01 to 1.50% of Cr can be added singly or in a mixture. However,

with adding amounts smaller than lower limits, the effect of improving the iron loss is small, while with adding amounts larger than upper limits, development of secondary recrystallized grains is suppressed to cause difficulties in obtaining a good iron loss. Therefore, any of these elements is preferably added within the above range.

#### Other Elements

The balance except the above-described contained elements is preferably composed of Fe and inevitable impurities.

Of the above slab components, Mn, Si, Cr, Sb, Sn, Cu, Mo, Ni, P and most of the nitride forming elements are substantially the same in the composition of the slab and the composition of the grain oriented electromagnetic steel sheet as a product. Among the other components, the C and Al contents of the product sheet are decreased to 50 ppm or less and 100 ppm or less, respectively, and the contents of the elements other than the above-described elements are also decreased to 50 ppm or less. The analytical limit value of each of the elements C, N, B, S and P is about 0.0001%, and the limit values of the other elements are about 0.001%.

Next, the production method is described.

A slab is produced from melted steel prepared to the above-described preferable composition by a conventional ingot-making method or continuous casting method. Alternatively, a thin cast slab of 100 mm or less in thickness may be produced directly by a direct casting method.

Although the slab is hot-rolled by a conventional heating method, the slab may be hot-rolled immediately after casting without heating. For the thin cast slab, hot rolling may be performed, or a subsequent step may be performed without hot rolling.

A general process for producing a grain oriented electromagnetic steel sheet uses a heating temperature (slab heating temperature) of above 1300 to 1450° C. before hot rolling, but in our process, the slab heating temperature (the rolling start temperature when the slab is rolled without heating after casting) may be a lower temperature, for example, 1200 to 1300° C. because there is no need to dissolve the inhibitor. Hot rolling may be performed according to a conventional method.

Then, the hot-rolled sheet is annealed according to demand. However, in order to highly develop the Goss structure in the product sheet, the hot-rolled annealing temperature is preferably 800° C. to 1050° C. This is because with a hot-rolled sheet annealing temperature of less than 800° C., the band structure produced in hot rolling remains, while with a hot-rolled sheet annealing temperature of over 1050° C., the grains after hot-rolled sheet annealing are significantly coarsened. In both cases, development of the Goss structure of the product sheet deteriorates, resulting in a decrease in the magnetic flux density.

After hot-rolled sheet annealing, cold rolling is performed to obtain a final thickness. In this step, cold rolling may be performed once to obtain the final thickness, or may be performed twice or more with intermediate annealing performed therebetween to obtain the final thickness.

In cold rolling, in order to develop the Goss structure, it is effective both to increase the rolling temperature to 100 to 250° C., and to perform aging once or several times in the temperature range of 100 to 250° C. during the course of cold rolling.

Then, recrystallization annealing is performed to decrease the C content to 60 ppm or less, which causes no magnetic aging, preferably 50 ppm or less, and more preferably 30 ppm or less.

Recrystallization annealing (primary recrystallization annealing) after final cold rolling (one time of cold rolling or final cold rolling of a plurality of times of cold rolling) is preferably performed in the range of 800 to 1000° C.

As the atmosphere of recrystallization annealing, for example, an inert atmosphere of a single gas such as a hydrogen atmosphere, a nitrogen atmosphere or an argon atmosphere, or an atmosphere of a mixture thereof may be used.

As the atmosphere of recrystallization annealing is preferably a dry atmosphere having a dew point of 40° C. or lower, preferably 0° C. or lower, and a low oxidizing or non-oxidizing atmosphere is preferably used. Under these atmospheric conditions, surface oxides such as the undercoating, the internal oxide layer, and the like can easily be eliminated.

15 Namely, under the above conditions, the formation of surface oxides such as  $\text{SiO}_2$  and the like is preferably suppressed as much as possible in order to maintain a smooth surface and obtain a good iron loss.

20 By using the above atmosphere, the formation of a hard coating on the surfaces of the electromagnetic steel sheet can be prevented in final annealing or the like, thereby significantly improving the punching quality.

Furthermore, a technique of increasing the Si amount by 25 a siliconizing method may be performed at any desired time after final cold rolling, for example, after final cold rolling, after recrystallization annealing or after final annealing.

Then, an annealing separator is applied according to demand. However, it is important to avoid using  $\text{MgO}$  which 30 reacts with silica to form forsterite.

Therefore, it is most preferable not to apply the annealing separator, but when the annealing separator is added, a material which does not react with silica, such as colloidal silica, alumina powder, BN powder or the like, is used.

35 In coating the separator, electrostatic coating is effective for suppressing the formation of oxides without taking in moisture.

Then, final annealing is performed to develop a secondary recrystallized structure.

40 In order to develop secondary recrystallization annealing and secure 10 ppm or more of solute nitrogen, it is effective that the atmosphere of final annealing contains nitrogen.

Also, in order to suppress the formation of oxides, a low 45 oxidizing or non-oxidizing atmosphere having a dew point of 40° C. or lower, preferably 0° C. or lower, is preferably used. This is because with an excessively high dew point, the surface oxides are excessively produced to deteriorate not only the iron loss but also the punching quality.

Furthermore, in order to generate secondary recrystallization, final annealing is preferably performed at 800° C. or higher. Since the rate of heating to 800° C. has less influence 50 on the magnetic properties except in the case described below, the heating rate may be set to any condition. The maximum ultimate temperature must be 1000° C. or lower, preferably 950° C. or lower, in order to form fine crystal grains having a grain diameter of 0.15 mm to 0.50 mm corresponding to a circle at a rate of 2 grains/cm<sup>2</sup> or more, preferably 50 grains/cm<sup>2</sup> or more, in the secondary recrystallized grains to decrease the iron loss.

60 Although the lower limit of the dew point in each annealing is not limited, the possible lower limit is generally about -50° C. from the viewpoint of the process.

When the steel slab has an Al content of over 100 ppm, in order to obtain the good iron loss, final annealing is 65 preferably performed under a further condition in which (1) the rate of heating from 300° C. to 800° C. is 5 to 100° C./h, and (2) the highest heating temperature is 800° C. or higher.

This method is particularly effective for the slab composition satisfying 0.0060% of C, 2.5 to 4.5% of Si, 0.50% or less of Mn and 50 ppm or less of O (% by mass), and the final annealing described below is preferably performed with a dew point of 0° C. or lower.

In this way, the grain oriented electromagnetic steel sheet can be produced, in which the secondary recrystallized grains are steadily grown, and hard coatings such as the forsterite undercoating and the like are not formed on the surfaces. When steel sheets are laminated to assemble an electric motor or transformer, it is effective to perform insulation coating on the surfaces of the steel sheets in order to improve the iron loss. Although the insulation coating is not limited, organic coating containing a resin is preferred for securing good punching quality or lubricity. However, when weldability is regarded as important, inorganic coating is applied.

Examples of such coatings include organic types such as acryl, epoxy, vinyl, phenol, styrene, and melamine resin coatings, and the like; and semi-organic types obtained by adding inorganic colloid, a phosphoric acid compound, a chromic acid compound or the like to the organic resins.

The coatings are generally formed by coating a treatment solution (a solution of the above coating component) and then baking the resultant coating in the temperature range of about 100 to 350° C.

#### (Second aspect—Operation)

A second aspect is described. First, an experiment leading to success is described (Experiment 2-1).

A steel slab having a composition free from inhibitor components and containing, by % by mass, 0.0025% of C, 3.4% of Si, 0.06% of Mn, Al and N decreased to 30 ppm and 12 ppm, respectively, and other components decreased to 30 ppm or less was produced by continuous casting. Then, the steel slab was heated to 1200° C., and then hot-rolled to form a hot-rolled sheet of 2.5 mm in thickness. The hot-rolled sheet was soaked at 950° C. for 1 minute in a nitrogen atmosphere, and then rapidly cooled.

Then, after a final thickness of 0.35 mm was obtained by cold rolling, recrystallization annealing was performed by soaking at 930° C. for 20 seconds in an atmosphere containing 50 vol % of hydrogen and 50 vol % of nitrogen and having a dew point of -30° C. Then, a sample to which an annealing separator was not applied, and a sample to which a slurry mixture of MgO and water was applied as an annealing separator were formed.

Then, final annealing was performed. In the final annealing, the temperature was increased from room temperature to 875° C. at a rate of 50° C./h in a nitrogen atmosphere having a dew point of -20° C., kept at this temperature for 50 hours, and then further increased to various temperatures at a rate of 25° C./h.

The thus-obtained product sheets (Al reduced to 10 ppm, N reduced to about 30 ppm, and other components being the same as or reduced to lower than the levels of the slab components) were measured with respect to iron loss ( $W_{15/50}$ ). For a comparison, the iron loss ( $W_{15/50}$ ) of a commercial grain oriented electromagnetic steel sheet having the same thickness was measured.

FIG. 8 shows the results of measurement of the relationship between the ultimate temperature of final annealing and the iron loss in each of the rolling direction and the direction perpendicular to the rolling direction. Although the ultimate temperature of final annealing of the commercial grain

oriented electromagnetic steel sheet is unknown, the ultimate temperature thereof is also shown in the figure (this applies to FIGS. 9 and 10).

This figure indicates that in the sample to which the annealing separator was not applied, the iron loss in the rolling direction is substantially constant with an ultimate temperature of final annealing of 875° C. or higher, while the iron loss in the direction perpendicular to the rolling direction is particularly good in the ultimate temperature range of 875 to 975° C., and abruptly deteriorates when ultimate temperature exceeds 975° C. However, even when the iron loss deteriorates, the iron loss is superior to that of the commercial grain oriented electromagnetic steel sheet.

On the other hand, in the sample to which MgO was applied as the annealing separator, particularly the iron loss in the direction perpendicular to the rolling direction is inferior to that of the sample to which the annealing separator was not applied, and the iron loss abruptly deteriorates when the ultimate temperature of final annealing exceeds 950° C., thereby obtaining only an iron loss close to the commercial grain oriented electromagnetic steel sheet.

FIG. 9 shows a comparison of the ratio of the iron loss in the direction perpendicular to the rolling direction to that in the rolling direction between presence and absence of the annealing separator.

As shown in the figure, the iron loss ratio of the commercial grain oriented electromagnetic steel sheet is about 4, exhibiting extremely high anisotropy. However, in the case of final annealing at 975° C. or lower without the annealing separator being applied, the iron loss ratio is 2.6 or less, and the anisotropy is significantly decreased as compared with the commercial grain oriented electromagnetic steel sheet. The significant improvement in the iron loss in the direction perpendicular to the rolling direction suggests that the samples are very useful as a material for an EI core affected by the iron loss in the direction perpendicular to the rolling direction, as compared with existing grain oriented electromagnetic steel sheets.

Next, in order to elucidate the reason why a good iron loss is obtained, particularly, in the direction perpendicular to the rolling direction to decrease the anisotropy of the iron loss when the annealing separator is not applied, the iron loss of each of the sample to which the annealing separator was applied, and the commercial grain oriented electromagnetic steel sheet was measured after the surface oxide coating was pickled, and then the surface was smoothed by electropolishing. The results are summarized in FIG. 10.

This figure indicates newly found matter that in both the sample to which the annealing separator was applied, and the commercial grain oriented electromagnetic steel sheet, the iron loss in the direction perpendicular to the rolling direction is improved by removing the oxide coating from the surface and further smoothing the surface.

As a result of the same treatment of the sample to which the annealing separator was not applied, the iron loss was little changed.

This result suggests that the forsterite undercoating formed on the surface of the steel sheet significantly deteriorates the iron loss in the direction perpendicular to the rolling direction.

Next, an examination was made of the crystal structure of the sample to which the annealing separator was not applied, and which exhibited a good iron loss with low anisotropy.

FIG. 11 shows the crystal structure after final annealing. This figure indicates that fine crystal grains having a grain diameter of about 0.15 to 0.50 mm are scattered in coarse secondary recrystallized grains of several cm. The existence

rate of the fine grains was determined by measuring the number of fine crystal grains in a 3-cm square region of the surface of the steel sheet.

It is thus found that the existence rate of fine crystal grains having a grain diameter of 0.15 to 0.50 mm and the iron loss in the direction perpendicular to the rolling direction have a strong correlation.

The fine grains decrease in number as the ultimate temperature of final annealing increases, and disappear at around 1050°C.

FIG. 12 shows the results of measurement of the relationship between the existence rate of fine grains and the ratio of the iron loss in the direction perpendicular to the rolling direction to that in the rolling direction.

The figure indicates that the iron loss in the direction perpendicular to the rolling direction is improved as the rate of the fine crystal grains increases. Namely, when the existence rate of the fine crystal grains having a grain diameter of 0.15 to 0.50 mm is 3 grains/cm<sup>2</sup> or more, preferably 10 grains/cm<sup>2</sup> or more, the iron loss in the direction perpendicular to the rolling direction is significantly improved.

When the ultimate temperature of final annealing is 1000°C. or lower, the secondary recrystallized grains contain 2 grains/cm<sup>2</sup> or more of fine crystal grains having a grain diameter of 0.15 mm to 0.50 mm and passing through the sheet in the thickness direction, and when the temperature is 975°C. or lower, 10 grains/cm<sup>2</sup> or more of fine grains can be secured.

Next, in order to obtain knowledge about an improvement in the magnetic flux density, experiment was carried out by changing the grain diameter before cold rolling under various hot-rolled sheet annealing conditions (Experiment 2-2).

A steel slab having a composition free from inhibitor components and containing, by % by mass, 0.023% of C, 3.4% of Si, 0.06% of Mn, Al and N decreased to 50 ppm and 22 ppm, respectively, and other components decreased to 30 ppm or less was produced by continuous casting. Then, the steel slab was heated to 1200°C., and then hot-rolled to form a hot-rolled sheet of 3.2 mm in thickness. The hot-rolled sheet was annealed at various temperatures for various soaking times in a nitrogen atmosphere, and then rapidly cooled.

Then, after cold rolling was performed at a temperature of 200°C. to obtain a final thickness of 0.30 mm, decarburization and recrystallization annealing was performed by soaking at 930°C. for 45 seconds in an atmosphere containing 50 vol % of hydrogen and 50 vol % of nitrogen and having a dew point of 35°C. Then, final annealing was performed without the annealing separator being applied. In the final annealing, the temperature was increased from room temperature to 875°C. at a rate of 50°C./h in a nitrogen atmosphere having a dew point of -20°C., and then kept at this temperature for 50 hours.

The thus-obtained product sheet (C decreased to 20 ppm, Al decreased to 20 ppm, N decreased to about 30 ppm, and other components being the same as or decreased to lower than the levels of the slab components) was measured with respect to the magnetic flux density ( $B_{50}$ ) and iron loss ( $W_{15/50}$ ).

In any of experimental materials, the secondary recrystallized grains contained fine crystal grains having grain diameter of 0.15 mm to 0.50 mm at a rate of 10 grains/cm<sup>2</sup> or more.

FIGS. 13 and 14 show the results of measurement of the relationship between the grain diameter (corresponding to a circle) before final cold rolling and the magnetic properties

(the magnetic flux density and iron loss) in the rolling direction and the direction perpendicular to the rolling direction.

As shown in FIG. 13, as the grains before cold rolling 5 coarsen, the magnetic flux density in the direction perpendicular to the rolling direction is improved to decrease the anisotropy of the magnetic flux densities in the rolling direction and the direction perpendicular to the rolling direction, exhibiting that  $B_{L50} \geq 1.85$  T and  $B_{C50} \geq 1.70$  T. As 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040

rolling direction cannot be made by domain wall motion of the 180° magnetic domains. When tensile force is applied to the surface of the steel sheet by the tensile coating and the forsterite undercoating, the 180° domain structure is stabilized, and consequently magnetization in the direction perpendicular to the rolling direction is inhibited, possibly deteriorating the iron loss in the direction perpendicular to the rolling direction.

Therefore, by removing the forsterite undercoating, the 180° domain structure is destabilized to promote magnetization in the direction perpendicular to the rolling direction, thereby possibly improving the iron loss in the direction perpendicular to the rolling direction.

Next, the reason why the iron loss is decreased by keeping down the ultimate temperature of final annealing to 975° C. or lower to leave the fine crystal grains is not made clear. However, the inventors consider the reason as follows.

Namely, as described above in the first aspect, the presence of the fine crystal grains in the secondary recrystallized grains possibly causes subdivision of the magnetic domains to decrease an eddy current loss. The conventional technique using the inhibitor can achieve a low iron loss only when the inhibitor components (S, Se, N and the like) are purified by annealing at a high temperature of about 1000<sup>20</sup> C. or higher. However, the method of present invention not using the inhibitor can achieve a low iron loss by completing secondary recrystallization without purification, and thus the method of keeping down the ultimate temperature of final annealing to 975° C. or lower to leave a desired amount of fine grains possibly effectively functions.

The possible reason why the magnetic flux density in the direction perpendicular to the rolling direction is improved by coarsening the grains before final cold rolling is that as the grains before cold rolling coarsen, the {111} structure as the primary recrystallized aggregate structure decreases, and {100} to {411} components increase instead of the {111} structure to mix the secondary recrystallized grains having {100}<001> orientation.

Finally, the reason why secondary recrystallization is developed in steel not containing the inhibitor components is considered as described above in the first aspect with reference to FIG. 7.

#### (Second Aspect—Limitation and Preferred Range)

Next, the reasons for limiting the features of the second aspect will be described.

First, the grain oriented electromagnetic steel sheet of the second aspect must contain as a component, by % by mass, 1.0 to 8.0% of, preferably 2.0 to 8.0% of, Si.

Like in the first aspect, this is because with a Si content of less than 1.0%, the sufficient effect of improving the iron loss cannot be obtained, while with a Si content of over 8.0%, processability deteriorates. To obtain the excellent effect of improving the iron loss, the Si content is preferably in the range of 2.0% to 8.0%.

For the same reason as the steel sheet of the first aspect, to decrease the iron loss, the secondary recrystallized grains must contain fine crystal grains having a grain diameter of 0.15 mm to 0.50 mm at a rate of 2 grains/cm<sup>2</sup> or more, preferably 50 grains/cm<sup>2</sup> or more. From the viewpoint of an improvement of anisotropy of the iron loss, the fine grains are present at a rate of 3 grains/cm<sup>2</sup> or more, preferably 10 grains/cm<sup>2</sup> or more. For the same reason as the first embodiment, the upper limit of the existence rate of the fine crystal grains is preferably about 1000 grains/cm<sup>2</sup>.

To secure the superiority in the iron loss value of the steel sheet to an existing non-oriented electromagnetic steel sheet

when the steel sheet is used for the EI core, the iron loss ( $W_{L15/50}$ ) value of the steel sheet in the rolling direction is 1.40 W/kg or less, the iron loss ( $W_{c15/50}$ ) of the steel sheet in the direction perpendicular to the rolling direction is 2.6 times or less as large as the iron loss ( $W_{L15/50}$ ) in the rolling direction.

In order to secure good punching quality, a major premise is that the undercoating mainly composed of forsterite ( $Mg_2SiO_4$ ) is not formed on the surface of the steel sheet.

Next, the limitations of the components of the raw material slab for producing the electromagnetic steel sheet will be described. The reasons for the limitations including the preferred ranges are the same as the first aspect. In the composition below, “%” is “% by mass”.

15 C: 0.08% or less, preferably 0.006% or less  
Mn: 0.005 to 3.0%, preferably 0.05% or less  
Si: 1.0 to 8.0%, preferably 2.0 to 8.0%

16 Al: 0.020% or less, preferably less than 150 ppm, more preferably 100 ppm or less

20 N: 50 ppm or less, preferably 30 ppm or less

Inhibitor forming elements (S, Se, and the like): B is 10 ppm or less, and other elements are 50 ppm or less, preferably 30 ppm or less.

25 Nitride forming elements (Ti, Nb, Ta, V and the like): It is effective to decrease to 50 ppm or less.

0: 50 ppm or less, preferably 30 ppm or less

Elements other than the essential components and the inhibited components, which can be appropriately added (singly or in a mixture) include the following: Ni: 0.005 to 1.50%, preferably 0.01% or more, Sn: 0.01 to 1.50%, Sb: 0.005 to 0.50%, Cu: 0.01 to 1.50%, P: 0.005 to 0.50%, Mo: 0.005 to 0.50%, Cr: 0.01 to 1.5%, etc.

The balance except the above contained elements is preferably composed of Fe and inevitable impurities. The influence of the composition on the grain oriented electromagnetic steel sheet (product) composition is as described above in the first aspect.

35 The production method will be described.

40 A slab is produced from molten steel prepared to the above preferable composition by the conventional ingot making method or continuous casting method. A thin cast slab having a thickness of 100 mm or less may be produced directly by a direct casting method.

45 The slab is hot-rolled by a usual heating method, but may be hot-rolled immediately after casting without heating. The thin cast slab may be hot-rolled or transferred to a subsequent step without hot rolling.

50 The preferred range of slab heating temperatures (rolling start temperatures in the case of rolling without heating after casting) is the same as the first embodiment of the present invention.

55 Then, hot-rolled sheet annealing is performed according to demand. The temperature of hot-rolled sheet annealing is advantageously 800° C. or higher which accelerates recrystallization. However, in order to improve the magnetic flux density in the direction perpendicular to the rolling direction, it is effective that the grain diameter before final cold

60 rolling (the one cold rolling or final cold rolling of a plurality of times of cold rolling) is 150  $\mu$ m or more for obtaining  $B_{c50} > 1.70$  T exceeding the level of an existing non-oriented electromagnetic steel sheet. In order to set the grain diameter before final cold rolling to 150  $\mu$ m or more, the temperature of annealing (hot-rolled sheet annealing or intermediate annealing) immediately before final cold rolling is preferably 1050° C. or higher.

After hot-rolled sheet annealing, cold rolling is preformed to obtain a final thickness. In this step, cold rolling may be performed by one step or two or more steps with intermediate annealing performed therebetween to obtain the final thickness.

During cold rolling, in order to develop the Goss orientation, it is effective both to increase the rolling temperature to 100 to 250° C., and to perform aging once or several times in the temperature range of 100 to 250° C. in the course of cold rolling.

Then, recrystallization annealing is performed to decrease the C content to 60 ppm or less, which causes no magnetic aging, preferably 50 ppm or less, and more preferably 30 ppm or less.

In recrystallization annealing (primary recrystallization annealing) after final cold rolling, the grain diameter after recrystallization annealing must be controlled in the range of 30 to 80  $\mu\text{m}$ . This is because with a grain diameter of less than 30  $\mu\text{m}$  after recrystallization annealing, secondary recrystallized grains with a low degree of orientation integration are produced to deteriorate the iron losses both in the rolling direction and the direction perpendicular to the rolling direction. On the other hand, with a grain diameter of over 80  $\mu\text{m}$  after recrystallization annealing, secondary recrystallization does not occur to significantly deteriorate both the iron loss and the magnetic flux density. As an economical method for controlling the grain diameter after recrystallization annealing to 30 to 80  $\mu\text{m}$ , it is recommended that recrystallization annealing is performed by soaking in the temperature range of 850 to 975° C. for a short time (60 to 360 seconds at 850° C., and about 5 to 10 seconds at 975° C. depending upon the annealing temperature). In the case of annealing at a lower temperature, annealing must be performed for a relatively long time (for example, about 10 to 3600 minutes at 800° C.).

The preferred atmosphere for recrystallization annealing is the same as the first embodiment.

Also, a technique for increasing the Si amount by a siliconizing method may be employed after final cold rolling or recrystallization annealing.

Then, the annealing separator is applied according to demand, paying attention to the same points as the first embodiment.

Then, final annealing is performed to develop secondary recrystallized structure. In order to develop secondary recrystallization, final annealing is preferably performed at 800° C. or higher. On the other hand, the maximum ultimate temperature is 975° C. or lower in order to obtain a stable state in which fine crystal grains having a grain diameter of 0.15 mm to 0.50 mm are scattered at a predetermined rate in secondary recrystallized grains resulting a stable improvement in iron loss in the direction perpendicular to the rolling direction.

The preferable conditions of the atmosphere and the heating rate of final annealing are the same as the first embodiment.

When steel sheets are laminated, it is effective to perform insulation coating on the surface of each steel sheet in order to improve the iron loss. The preferable coating and coating method are the same as the first embodiment.

#### (Third Aspect—Operation)

A third aspect is described. First, experiment resulting in the success of the third aspect is described (Experiment 3-1).

A steel slab having a composition free from inhibitor components and containing, by % by mass, 0.0025% of C, 3.5% of Si, 0.04% of Mn, Al and N decreased to 50 ppm and

10 ppm, respectively, and other components reduced to 30 ppm or less was produced by continuous casting. Then, the steel slab was heated to 1250° C., and then hot-rolled to form a hot-rolled sheet of 1.6 mm in thickness. The hot-rolled sheet was soaked at 850° C. for 60 seconds in a nitrogen atmosphere, and then rapidly cooled. Then, after a final thickness of 0.20 mm was obtained by cold rolling, recrystallization annealing was performed by soaking at 920° C. for 10 seconds in an atmosphere containing 50 vol % of hydrogen and 50 vol % of nitrogen and having a dew point of -30° C.

Then, a sample to which the annealing separator was not applied, and a sample to which a slurry mixture containing MgO and water was applied as the annealing separator were formed, and these samples was subjected to final annealing. In the final annealing, the temperature was increased from room temperature to 850° C. at a rate of 50° C./h in a nitrogen atmosphere having a dew point of -20° C., kept at this temperature for 50 hours, and then further increased to various temperatures at a rate of 25° C./h.

The thus-obtained sheet products (Al decreased to 30 ppm, N decreased to about 20 ppm, and other components being the same as or decreased to lower than the levels of the slab components) were examined with respect to the iron loss  $W_{10/1000}$  (the iron loss by excitation to 1.0 T at a frequency of 1000 Hz). FIG. 15 shows the relationship between the measured iron loss and the ultimate temperature of final finish annealing.

For comparison, FIG. 15 also shows the results of measurement of the iron losses ( $W_{10/1000}$ ) of a commercial grain oriented electromagnetic steel sheet and a non-oriented electromagnetic steel sheet. Although the ultimate temperatures of final annealing of the commercial grain oriented electromagnetic steel sheet and the non-oriented electromagnetic steel sheet are not known, the ultimate temperatures are shown on the right ordinate of the figure.

The figure indicates that in the sample to which the annealing separator was not applied, a good iron loss is obtained when the ultimate temperature of final annealing is in the range of 850 to 950° C., and the iron loss deteriorates when the ultimate temperature exceeds 1000° C.

On the other hand, in the sample to which MgO was applied as the annealing separator, the iron loss at 1000 Hz is inferior to the sample to which the annealing separator was not applied, regardless of the ultimate temperature of final annealing, and the iron loss is equivalent to the commercial grain oriented electromagnetic steel sheet at the best.

Next, in order to elucidate the reason why the good iron loss at high frequency is obtained when the annealing separator is not applied, the sample to which the annealing separator was not applied and the sample to which MgO was applied as the annealing separator, both samples exhibiting the ultimate temperature of final annealing of 850° C. in the above experiment, and the commercial grain oriented electromagnetic steel sheet were measured with respect to the iron loss  $W_{17/50}$  at commercial frequency and the iron loss  $W_{10/1000}$  at high frequency after the surface oxide coating of each sample was removed by chemical polishing with hydrofluoric acid, and the surface of each sample was smoothed. Comparison of the results is shown in FIGS. 16(a) and (b).

As shown in the figures, in the sample to which the annealing separator was applied, the iron loss at a high frequency of 1000 Hz is significantly improved by removing the surface oxide coating and smoothing the surface, obtaining a good value close to that of the sample to which the annealing separator was not applied. In the grain oriented

electromagnetic steel sheet, the iron loss at high frequency is slightly improved by removing the surface oxide coating.

However, in the sample to which the annealing separator was applied, the iron loss at high frequency is substantially the same before and after removal of the surface oxide coating.

The results shown in FIG. 16 suggest that the iron loss at high frequency is significantly deteriorated by the oxide coating formed on the surface of the steel sheet. Also, a comparison of the iron losses after removal of the oxide coating shows that the iron losses of the samples of this experiment are superior to that of the commercial grain oriented electromagnetic steel sheet.

In this experiment, the surfaces of the samples were finished to mirror surfaces by electropolishing, and thus it was found that an iron loss improving factor other than the surface state is present.

Therefore, in order to find the factor, the sample to which the annealing separator was not applied, and which exhibited a good iron loss at high frequency was examined with respect to its crystal structure.

FIG. 17 shows the result of examination of the crystal structure after retention at 850° C.

This figure indicates that fine crystal grains having a grain diameter of about 0.15 to 1.00 mm are scattered in secondary recrystallized coarse grains of as large as several cm.

It is also found that the existence rate of the fine crystal grains having a grain diameter in the range of about 0.15 to 1.00 mm has a strong correlation with the iron loss at high frequency.

FIG. 18 shows the results of examination of the relationship between the existence rate of fine grains and the high-frequency iron loss ( $W_{10/1000}$ ). The existence rate of fine grains was determined by measuring the number of fine crystal grains having a grain diameter (corresponding to a circle) of 0.15 to 1.00 mm in a 3-cm square region of the surface of the steel sheet.

As shown in the figure, it is newly recognized that the high-frequency iron loss ( $W_{10/1000}$ ) is significantly improved as the existence rate of fine crystal grains in the secondary recrystallized grains increases to, particularly, 10 grains/cm<sup>2</sup> or more.

When the ultimate temperature of final annealing is 975° C. or lower, the fine crystal grains having a grain diameter of 0.15 mm to 0.50 mm are present in the secondary recrystallized grains at a rate of 2 grains/cm<sup>2</sup> or more (because the final annealing temperature is lower than 1000° C.). However, in the third aspect, the grain diameter of 0.15 mm to 1.00 mm is used as an index because the existence rate of the fine crystal grains having the grain diameter of 0.15 mm to 1.00 mm is thought to have a good correlation with the property concerned.

Next, in order to obtain knowledge about proper control of the production conditions for improving the high-frequency iron loss, the relationship between the high-frequency iron loss and the area ratio of Goss orientation grains, and the influence of the crystal grain diameter before cold rolling on the area ratio of Goss orientation grains were examined (Experiment 3-2).

The crystal grain diameter before cold rolling was changed to various values by changing the hot-rolled sheet annealing conditions. The area ratio of Goss orientation grains represents the existence rate of crystal grains with a shift angle of 20° or less from Goss orientation.

Namely, a steel slab having a composition free from inhibitor components and containing, by % by mass, 0.003% of C, 3.4% of Si, 0.06% of Mn, Al and N decreased to 50

ppm and 22 ppm, respectively, and other components reduced to 30 ppm or less was produced by continuous casting. Then, the steel slab was heated to 1200° C., and then hot-rolled to form a hot-rolled sheet of 1.6 mm in thickness.

The hot-rolled sheet was annealed at various temperatures for various soaking times in a nitrogen atmosphere, and then rapidly cooled. Then, the grain diameter was measured before final cold rolling, and then cold rolling was performed to obtain a final thickness of 0.20 mm.

Then, recrystallization annealing was performed by soaking at 930° C. for 15 seconds in an atmosphere containing 50 vol % of hydrogen and 50 vol % of nitrogen and having a dew point of -50° C., and final annealing was performed without the annealing separator being applied. In the final annealing, the temperature was increased from room temperature to 875° C. at a rate of 50° C./h in a nitrogen atmosphere having a dew point of -20° C., and kept at this temperature for 50 hours.

The thus-obtained product sheets (Al decreased to 30 ppm, N decreased to about 25 ppm, and the other components being the same as or decreased to lower than the levels of the slab) were measured with respect to the area ratio of Goss orientation and the high-frequency iron loss ( $W_{10/1000}$ ).

In any of experimental materials, the secondary recrystallized grains contained fine crystal grains having a grain diameter of 0.15 mm to 0.50 mm at a rate of 2 grains/cm<sup>2</sup> or more, and fine crystal grains having a grain diameter of 0.15 mm to 1.00 mm at a rate of 10 grains/cm<sup>2</sup> or more.

FIG. 19 shows the relationship between the high-frequency iron loss ( $W_{10/1000}$ ) and the area ratio of Goss orientation grains.

As shown in this figure, a high-frequency iron loss superior to the commercial grain oriented electromagnetic steel sheet is obtained when the area ratio of Goss orientation grains is 50% or more.

FIG. 20 shows the relationship between the grain diameter before cold rolling and the area ratio of Goss orientation grains. As shown in this figure, an area ratio of Goss orientation grains of 50% or more is secured when the grain diameter before cold rolling is less than 150 µm.

As a result, it is found that as a preferred production condition for obtaining a good high-frequency iron loss, the grain diameter before final cold rolling must be less than 150 µm.

When the above experimental results are summarized, it is found that by using a high-purity raw material not containing the inhibitor, suppressing the formation of a forsterite undercoating in final annealing to form a smooth surface, and keeping down the ultimate temperature of final annealing to 975° C. or lower to leave fine crystal grains in secondary recrystallized grains, the high-frequency iron loss is significantly improved, as compared with a conventional grain oriented electromagnetic steel sheet.

It is also found that in order to secure an area ratio of Goss orientation grains of 50% or more to obtain a good high-frequency iron loss, it is effective to set a grain diameter before final cold rolling to less than 150 µm.

Although the reason for the first finding leading to the success, i.e., the reason why the high-frequency iron loss is improved by avoiding applying the annealing separator or by not using MgO as the annealing separator to remove the formation of the forsterite undercoating, is not always known, we consider the reason as follows.

MgO generally used as the annealing separator reacts at high temperature with SiO<sub>2</sub> formed in decarburization annealing and final annealing to form the forsterite (Mg<sub>2</sub>SiO<sub>4</sub>) undercoating on the surface of the steel sheet,

and functions to secure adhesion to tensile coating mainly composed of a phosphate or the like. The interface between the forsterite undercoating and the base metal is a portion generally referred to as an "anchor portion" in which an oxide is mixed with the base metal in a complicated form. This complicated structure is effective for securing adhesion to the tensile coating mainly composed of a phosphate or the like, but significantly deteriorates smoothness of the base metal surface.

Magnetization in a high-frequency region produces a skin effect in which magnetization on the surface preferentially occurs, as compared with magnetization at the commercial frequency. It is thus presumed that the high-frequency iron loss is good with a highly smooth surface free from the forsterite undercoating.

Next, the reason why the iron loss is decreased by keeping down the ultimate temperature of final annealing to 975°C. or lower to leave fine crystal grains is not always known, but the inventors consider the reason as follows.

As described above in the first and second aspects, the presence of fine crystal grains in secondary recrystallized grains possibly causes subdivision of magnetic domains to decrease the eddy current loss. The conventional technique using the inhibitor can achieve a low iron loss only when the inhibitor components (S, Se, N and the like) are purified by annealing at high temperature of about 1000°C. or higher. However, the method of the present invention not using the inhibitor can achieve a low iron loss only by completing secondary recrystallization without purification, and thus the method of keeping down the ultimate temperature of finish annealing to leave a desired amount of fine grains which pass through the sheet in the thickness direction is possibly effectively functions.

The conceivable reason why the area ratio of Goss orientation grains is increased to improve the high-frequency iron loss by suppressing coarsening of the grains before final cold rolling is that the degree of accumulation of {111} structure in the primary recrystallized texture is increased by keeping the grains fine before cold rolling, forming the primary recrystallized texture useful for growth of Goss orientation recrystallized grains.

The reason why secondary recrystallization is developed in steel not containing the inhibitor components is considered as described above in the first aspect with reference to FIG. 7.

#### (Third Aspect—Limitation and Preferred Range)

The reasons for limiting the features of the third aspect will be described.

First, the electromagnetic steel sheet must contain as a component, by % by mass, 1.0 to 8.0% of, preferably 2.0 to 8.0% of, Si.

Like in the first aspect, this is because with a Si content of less than 1.0%, the sufficient effect of improving the iron loss cannot be obtained, while with a Si content of over 8.0%, processability deteriorates. To obtain the excellent effect of improving the iron loss, the Si content is preferably in the range of 2.0% to 8.0%.

Furthermore, it is necessary that the grain diameter of the secondary recrystallized grains on the surface of the steel sheet, which is measured except fine grains having a grain diameter of 1 mm or less, is 5 mm or more. This is because when the secondary recrystallized grains have a grain diameter of less than 5 mm, the area ratio of Goss orientation grains is decreased to fail to obtain a good high-frequency iron loss. In order to set the grain diameter of the secondary recrystallized grains to 5 mm or more, it is preferable to

sufficiently decrease impurity elements, obtain a grain diameter of 30 to 80  $\mu\text{m}$  after recrystallization annealing, and stay the grains in the temperature region of 800°C. or higher for 30 hours or more during final annealing. By satisfying these conditions, the secondary recrystallized grains can be sufficiently developed to achieve an average grain diameter of 5 mm or more.

Furthermore, in the steel sheet to decrease the high-frequency iron loss, the secondary recrystallized grains must contain fine crystal grains having a grain diameter of 0.15 mm or 1.0 mm at a rate of 10 grains/cm<sup>2</sup> or more.

Under the production conditions for obtaining the above fine grain distribution, it is possible to achieve the state in which the secondary recrystallized grains contain fine crystal grains having a grain diameter of 0.15 mm to 0.50 mm at a rate of 2 grains/cm<sup>2</sup> or more, preferably 50 grains/cm<sup>2</sup> or more. This is effective for decreasing the iron loss for the same reason as the steel sheet of the first embodiment. The upper limit of the existence rate of the fine grains (grain diameter of 0.15 mm to 0.50 mm) is preferably about 1000 grains/cm<sup>2</sup> for the same reason as the first aspect.

The upper limit of the existence rate of fine grains having a grain diameter of 0.15 mm to 1.00 mm is preferably about 500 grains/cm<sup>2</sup>.

With the fine grains having a grain diameter of less than 0.15 mm or over 1.00 mm, the effect of subdividing the magnetic domains is small, causing no contribution to a decrease in the iron loss. Therefore, the existence rate of fine crystal grains having a grain diameter in the range of 0.15 to 1.00 mm is taken into consideration. However, when the existence rate of the fine crystal grains is less than 10 grains/cm<sup>2</sup>, the effect of subdividing the magnetic domains is decreased to fail to expect a sufficient improvement in the high-frequency iron loss.

In order to obtain a good high-frequency iron loss, it is also an essential condition that the area ratio of grains with an orientation shift angle of 20° or less from {110}<001> orientation, i.e., the area ratio of Goss orientation grains, is 50% or more, preferably 80% or more.

This is because when the area ratio of Goss orientation grains is less than 50%, the high-frequency iron loss is equivalent to an existing grain oriented electromagnetic steel sheet to lose the advantage of the electromagnetic steel sheet.

Furthermore, a main premise is that the undercoating mainly composed of forsterite ( $\text{Mg}_2\text{SiO}_4$ ) is not formed on the surface of the steel sheet in order to form a magnetically smooth plane and secure a good high-frequency iron loss.

Next, the limitations of the components of the raw material slab for producing the electromagnetic steel sheet will be described. The reasons for the limitations including the preferred ranges are the same as the first aspect. In the composition below, "%" is "% by mass".

C: 0.08% or less, preferably 0.006% or less

In the third aspect, the surface smoothness of the product is very important, and thus C is more preferably 50 ppm or less.

Mn: 0.005 to 3.0%, preferably 0.50% or less

Si: 1.0 to 8.0%, preferably 2.0 to 8.0%

Al: 0.020% or less, preferably less than 150 ppm, more preferably 100 ppm or less

N: 50 ppm or less, preferably 30 ppm or less

Inhibitor components (S, Se, and the like): B is 10 ppm or less, and the other components are 50 ppm or less, preferably 30 ppm or less.

## 31

Nitride forming elements (Ti, Nb, Ta, V and the like): An amount of 50 ppm or less is effective.

O: 50 ppm or less, preferably 30 ppm or less

Elements other than the above necessary components and the inhibited components, which can be appropriately added (singly or in a mixture) include the following:

Ni: 0.005 to 1.50%, preferably 0.01% or more, Sn: 0.01 to 1.50%, Sb: 0.005 to 0.50%, Cu: 0.01 to 1.50%, P: 0.005 to 0.50%, Mo: 0.005 to 0.50%, Cr: 0.01 to 1.5%, etc.

These elements exhibit the effect of improving not only the iron loss at a usual frequency but also the iron loss at a high frequency in the above preferred ranges.

The balance except the above contained elements is preferably composed of Fe and inevitable impurities. The influence of the composition on the grain oriented electromagnetic steel sheet (product) composition is as described above in the first embodiment.

The production method will be described.

A slab is produced from molten steel prepared to the above preferable composition by the conventional ingot making method or continuous casting method. A thin cast slab having a thickness of 100 mm or less may be produced directly by a direct casting method.

The slab is hot-rolled by a usual heating method, but may be hot-rolled immediately after casting without heating. The thin cast slab may be hot-rolled or transferred to a subsequent step without hot rolling.

The preferred range of slab heating temperatures (rolling start temperatures in the case of rolling without heating after casting) is the same as the first aspect.

Then, hot-rolled sheet annealing is performed according to demand. The temperature of hot-rolled sheet annealing is favorably 800° C. or higher which accelerates recrystallization. However, in order to improve the high-frequency iron loss by securing an area ratio of 50% or more for crystal grains with an orientation shift of 20° or less from {110}<001> orientation, it is effective that the grain diameter before final cold rolling (the one cold rolling or final cold rolling of a plurality of times of cold rolling) is less than 150 µm, preferably 120 µm or less, for obtaining a high-frequency iron loss superior to the level of an existing grain oriented electromagnetic steel sheet. In order to set the grain diameter before final cold rolling to less than 150 µm, the temperature of annealing (hot-rolled sheet annealing or intermediate annealing) immediately before final cold rolling is preferably 1000° C. or lower.

After hot-rolled sheet annealing, cold rolling is performed to obtain a final thickness. In this step, cold rolling may be performed by one step, or two or more steps with intermediate annealing performed therebetween to obtain the final thickness.

During cold rolling, in order to develop the Goss orientation, it is effective both to increase the rolling temperature to 100 to 250° C., and to perform aging once or several times in the temperature range of 100 to 250° C. in the course of cold rolling.

Then, recrystallization annealing is performed to decrease the C content to 60 ppm or less, which causes no magnetic aging, preferably 50 ppm or less, and more preferably 30 ppm or less.

In recrystallization annealing (primary recrystallization annealing) after final cold rolling, the grain diameter after recrystallization annealing must be controlled in the range of 30 to 80 µm. This is because with a grain diameter of less than 30 µm after recrystallization, secondary recrystallized grains having an orientation apart from Goss orientation are produced to deteriorate the high-frequency iron loss. On the

## 32

other hand, with a grain diameter of over 80 µm after recrystallization annealing, secondary recrystallization does not occur to deteriorate the high-frequency iron loss. In order to control the grain diameter after recrystallization annealing to 30 to 80 µm, it is economically advantageous that recrystallization annealing is continuously performed by soaking in the temperature range of 850 to 975° C. for a short time (refer to the description of the second embodiment).

10 The preferred atmosphere of recrystallization annealing is the same as the first aspect.

Also, a technique for increasing the Si amount by a siliconizing method may be employed after final cold rolling or recrystallization annealing.

15 Then, the annealing separator is applied according to demand, paying attention to the same points as the first aspect.

Then, final annealing is performed to develop a secondary recrystallized structure. In order to develop secondary recrystallization, final annealing is preferably performed at 800° C. or higher. On the other hand, the maximum ultimate temperature is 975° C. or lower in order to obtain a state in which fine crystal grains having a grain diameter of 0.15 mm to 1.00 mm are scattered at a desired distribution rate in secondary recrystallized grains, improving the high-frequency iron loss.

The preferable conditions of the atmosphere and the heating rate of final annealing are the same as the first aspect.

When steel sheets are laminated, it is effective to perform insulation coating on the surface of each steel sheet in order to improve the iron loss. The preferable coating and coating method are the same as the first embodiment.

Although the requirements and the preferred conditions of each of the first to third aspect are described separately, the requirements or the preferred conditions of the first aspect may be applied to the second or third aspect (within a range not interdicting with the object). Similarly, the requirements or the preferred conditions of the second aspect may be freely applied to the first or third aspect, and the requirements or the preferred conditions of the third aspect may be freely applied to the first or second aspect.

## EXAMPLES

## Example 1

## First Aspect

A steel slab having a composition free, from inhibitor components and containing 0.002% of C, 3.4% of Si, 0.07% of Mn, 0.03% of Sb, Al and N decreased to 30 ppm and 9 ppm, respectively, and other components reduced to 50 ppm or less was produced by continuous casting. Then, the steel slab was heated at 1100° C. for 20 minutes, and then hot-rolled to form a hot-rolled sheet of 2.6 mm in thickness. The hot-rolled sheet was annealed by soaking at 800° C. for 60 seconds. Then, cold rolling was performed at 150° C. to obtain a final thickness of 0.30 mm.

Then, recrystallization annealing was performed by soaking at 930° C. for 10 seconds in an atmosphere containing 75 vol % of hydrogen and 25 vol % of nitrogen and having each of the various dew points shown in Table 2. Then, final annealing was performed under a condition in which the temperature was increased to 800° C. at a rate of 50° C./h in a mixed atmosphere (dew point -30° C.) containing 50 vol % of nitrogen and 50 vol % of Ar, further increased from 800° C. to 900° C. at a rate of 10° C./h, and maintained at

this temperature for 30 hours. After final annealing, the N amount of steel was 33 ppm and the Al amount was 5 ppm.

Then, the finish annealed sheet was coated with a coating solution made by mixing aluminum bichromate, an emulsion resin and ethylene glycol, and baked at 300° C. to form a product.

An EI core was formed from the thus-obtained product sheet by punching, and measured with respect to its iron loss ( $W_{13/50}$ ).

Also, the existence rate of fine crystal grains having a grain diameter of 0.05 to 0.50 mm in the product sheet was determined by measuring the number of the fine crystal grains in a 3-cm square region on the surface of the steel sheet.

Furthermore, in order to evaluate punching quality, continuous punching into a 17-mm square was carried out by using a 25-ton press (material: SKD-11) and commercial punching oil under conditions of a punching rate of 350 strokes/min and a clearance of 6% of thickness until the burr height reached 50  $\mu$ m.

The obtained results are shown in Table 2.

| No. | Dew point of recrystallization annealing atmosphere (° C.) | EI core loss $W_{13/50}$ (W/kg) | Number of fine grains (/cm <sup>2</sup> ) | Number of times of punching (10,000 times) | Remarks             |
|-----|------------------------------------------------------------|---------------------------------|-------------------------------------------|--------------------------------------------|---------------------|
| 1   | -50                                                        | 0.81                            | 65.6                                      | >300                                       | Example             |
| 2   | -25                                                        | 0.82                            | 68.4                                      | >300                                       | Example             |
| 3   | 0                                                          | 0.83                            | 69.0                                      | >300                                       | Example             |
| 4   | 20                                                         | 0.85                            | 70.6                                      | 250                                        | Example             |
| 5   | 40                                                         | 0.90                            | 72.3                                      | 200                                        | Example             |
| 6   | 50                                                         | 0.99                            | 73.4                                      | 120                                        | Comparative example |
| 7   | 60                                                         | 1.03                            | 74.0                                      | 80                                         | Comparative example |

As shown in Table 2, when the dew point of the recrystallization annealing atmosphere is 40° C. or lower, particularly, 0° C. or lower, a product having both excellent punching quality and iron loss is obtained.

Example 2

First Aspect

5 A steel slab having a composition free from inhibitor components and containing 0.003% of C, 3.3% of Si, 0.52% of Mn, 0.08% of Cu, Al and N decreased to 50 ppm and 12 ppm, respectively, and other components reduced to 50 ppm or less was produced by continuous casting. Then, the steel slab was heated at 1200° C. for 20 minutes, and then hot-rolled to form a hot-rolled sheet of 2.2 mm in thickness. Then, the hot-rolled sheet was annealed at 900° C. for 20 seconds, and first cold rolling was performed at room temperature to obtain a thickness of 1.5 mm. After intermediate annealing at 950° C. for 30 seconds, second cold rolling was performed at room temperature under a condition in which aging was performed at 200° C. for 5 hours when the thickness was 0.90 mm in the course of cold 10 rolling, to finish the sheet to a final thickness of 0.27 mm.

15 Furthermore, in order to evaluate punching quality, continuous punching into a 17-mm square was carried out by using a 25-ton press (material: SKD-11) and commercial punching oil under conditions of a punching rate of 350 strokes/min and a clearance of 6% of thickness until the burr height reached 50  $\mu$ m.

20 Then, recrystallization annealing was performed by soaking at 900° C. for 30 seconds in an atmosphere containing 75 vol % of hydrogen and 25 vol % of nitrogen and having a dew point of -40° C. Then, final annealing was performed under a condition in which the temperature was increased from room temperature to 900° C. at a rate of 30° C./h in each of the atmospheres shown in Table 3, and maintained at this temperature for 50 hours. After final annealing, the Al 25 amount of steel was 30 ppm.

25 Then, the finish annealed sheet was coated with a coating solution made by mixing aluminum bichromate, an emulsion resin and ethylene glycol, and baked at 300° C. to form a product.

30 The thus-obtained product sheet was measured with respect to its iron loss ( $W_{17/50}$ ) in an EI core formed from the sheet by punching, the existence rate of fine crystal grains having a grain diameter of 0.15 to 0.50 mm in the product sheet, and the number of times of continuous punching until the burr height reached 50  $\mu$ m by the same method as 35 Example 1. The obtained results are shown in Table 3.

TABLE 3

| No. | Final finish annealing       |                  | N content of steel (ppm) | $W_{17/50}$ (W/kg) | Number of fine grains (10,000 times) | Number of times of punching (10,000 times) | Remarks             |
|-----|------------------------------|------------------|--------------------------|--------------------|--------------------------------------|--------------------------------------------|---------------------|
|     | Atmosphere (vol %)           | Dew point (° C.) |                          |                    |                                      |                                            |                     |
| 1   | Nitrogen: 50<br>Hydrogen: 50 | -30              | 44                       | 1.21               | 65.6                                 | >300                                       | Example             |
| 2   | Nitrogen: 100                | -30              | .64                      | 1.23               | 55.4                                 | >300                                       | Example             |
| 3   | Nitrogen: 25<br>Ar: 75       | -30              | 35                       | 1.22               | 65.6                                 | >300                                       | Example             |
| 4   | Nitrogen: 10<br>Hydrogen: 90 | -30              | 16                       | 1.20               | 76.0                                 | 270                                        | Example             |
| 5   | Nitrogen: 100                | 0                | 69                       | 1.36               | 59.2                                 | 220                                        | Example             |
| 6   | Nitrogen: 100                | 50               | 75                       | 1.50               | 61.9                                 | 150                                        | Comparative example |
| 7   | Hydrogen: 100                | -10              | 6                        | 1.56               | 89.2                                 | 120                                        | Comparative example |

As shown in Table 3, when the dew point of the atmosphere is 40° C. or lower, and the N amount of steel is 10 ppm or more, a product having both excellent punching quality and iron loss is obtained.

### Example 3

#### First Aspect

A steel slab having each of the compositions shown in Table 4 was heated to 1160° C., and then hot-rolled to form a hot-rolled sheet of 3.2 mm in thickness. All components other than those shown in Table 4 were decreased to 50 ppm or less, and the inhibitor components were not contained.

Then, the hot-rolled sheet was annealed by soaking at 1000° C. for 60 seconds, and then finished to a final thickness of 0.50 mm by cold rolling. Then, recrystallization annealing was performed by soaking at 980° C. for 20 seconds in an atmosphere containing 75 vol % of hydrogen and 25 vol % of nitrogen and having a dew point of -35° C. Then, final annealing was performed under a condition in which the temperature was increased to 850° C. at a rate of 10° C./h., and maintained at this temperature for 75 hours in a nitrogen atmosphere having a dew point of -40° C. In the examples, the Al amount of steel after final annealing was 5 to 40 ppm.

Then, the finish annealed sheet was coated with a coating solution made by mixing aluminum bichromate, an acrylic emulsion resin and boric acid, and baked at 300° C. to form a product.

The thus-obtained product sheet was measured with respect to its iron loss ( $W_{15/50}$ ) in an EI core formed from the sheet by punching, the existence rate of fine crystal grains having a grain diameter of 0.15 to 0.50 mm in the product sheet, and the number of times of continuous punching until the burr height reached 50  $\mu\text{m}$  by the same method as Example 1. The obtained results are shown in Table 4.

As shown in Table 4, by using a slab having a composition satisfying 0.003 to 0.08% of C, 2.0 to 8.0% of Si, 100 ppm or less of Al and 50 ppm or less of N, a product having excellent punching quality and iron loss is obtained.

Such a product is composed of steel containing 10 ppm or more of N, and contains secondary recrystallized grains having fine crystal grains having a diameter of 0.15 mm to 0.50 mm corresponding to a circle diameter at a rate of 2 grains/cm<sup>2</sup> or more.

#### (Example 4

#### First Aspect

Steel slabs A to D and Z each containing the components shown in Table 5 and a balance substantially composed of Fe (30 ppm or less each of other impurities, and without the inhibitor components) were produced by continuous casting, and heated at 1200° C. for 20 minutes. Then, each of the steel slabs was finished to a hot-rolled sheet of 2.6 mm in thickness by hot rolling. Then, each of the hot-rolled sheets was annealed (at 950° C. for 60 seconds), and finished to a final thickness of 0.35 mm by cold rolling. The S amount was lower than a level allowing S to function as the inhibitor. This applies to the examples below.

Among the steel slabs shown in Table 5, for steel slabs A to D, recrystallization annealing (primary recrystallization annealing) (at 930° C. for 10 seconds) was performed by a hydrogen atmosphere (a dew point of -20° C. or lower), and then final annealing (secondary recrystallization annealing) was performed at an annealing temperature of 920° C. in a nitrogen atmosphere (a dew point of -20° C.) without the annealing separator being applied. In this final annealing, the rate of heating from 300° C. to 800° C. was 20° C./h. In this example, after final annealing, the Al amount of steel was 5 to 60 ppm, and the S amount was 5 to 20 ppm.

TABLE 4

| No. | C  | Si   | Mn   | Ni   | Sn   | Sb   | Cu   | P    | Cr   | Mo | Al   | N  | (W/kg) | Number of fine grains (/cm <sup>2</sup> ) | N content (ppm) | Number of times of punching (10,000) | Chemical composition (mass %, ppm) |                    |
|-----|----|------|------|------|------|------|------|------|------|----|------|----|--------|-------------------------------------------|-----------------|--------------------------------------|------------------------------------|--------------------|
|     |    |      |      |      |      |      |      |      |      |    |      |    |        |                                           |                 |                                      | El core                            | W <sub>15/50</sub> |
| 1   | 23 | 3.44 | 0.13 | tr   | tr   | tr   | tr   | tr   | tr   | tr | 15   | 15 | 1.55   | 94.5                                      | 55              | >300                                 | Example                            |                    |
| 2   | 33 | 3.62 | 0.15 | 0.25 | tr   | tr   | tr   | tr   | tr   | tr | 37   | 23 | 1.50   | 86.7                                      | 60              | >300                                 | Example                            |                    |
| 3   | 24 | 3.47 | 0.25 | tr   | 0.10 | tr   | tr   | tr   | tr   | tr | 30   | 9  | 1.47   | 100.3                                     | 41              | >300                                 | Example                            |                    |
| 4   | 30 | 3.35 | 0.15 | tr   | tr   | 0.04 | tr   | tr   | tr   | tr | 55   | 12 | 1.47   | 50.3                                      | 33              | >300                                 | Example                            |                    |
| 5   | 35 | 3.52 | 0.03 | tr   | tr   | tr   | 0.10 | tr   | tr   | tr | 10   | 6  | 1.49   | 56.9                                      | 43              | >300                                 | Example                            |                    |
| 6   | 36 | 3.45 | 0.10 | tr   | tr   | tr   | tr   | 0.05 | tr   | tr | 32   | 15 | 1.55   | 90.5                                      | 48              | >300                                 | Example                            |                    |
| 7   | 16 | 3.22 | 0.07 | tr   | tr   | tr   | tr   | tr   | 0.50 | tr | 66   | 10 | 1.50   | 92.2                                      | 65              | >300                                 | Example                            |                    |
| 8   | 24 | 3.33 | 0.15 | tr   | tr   | tr   | tr   | tr   | tr   | tr | 150  | 20 | 1.83   | 143.5                                     | 120             | 140                                  | Comparative example                |                    |
| 9   | 15 | 3.30 | 0.19 | tr   | tr   | tr   | tr   | tr   | tr   | tr | 50   | 78 | 1.93   | 151.0                                     | 114             | 120                                  | Comparative example                |                    |
| 10  | 45 | 2.6  | 0.48 | tr   | 0.02 | 0.02 | tr   | tr   | tr   | tr | 24   | 11 | 1.65   | 75.5                                      | 28              | >300                                 |                                    |                    |
| 11  | 15 | 4.4  | 0.03 | tr   | tr   | 0.02 | 0.05 | 0.01 | tr   | tr | 23   | 12 | 1.37   | 102.4                                     | 23              | >300                                 |                                    |                    |
| 12  | 24 | 3.40 | 0.20 | tr   | tr   | tr   | tr   | tr   | tr   | tr | 0.02 | 30 | 15     | 1.51                                      | 85.3            | 30                                   | >300                               |                    |

In the table, C, Al and N are shown by ppm

In order to evaluate the punching quality of the thus-obtained steel sheets, a punching work was repeated by using a steel die having a diameter of 5 mm to evaluate the punching quality based on the number of times of punching until the burr height reached 50  $\mu\text{m}$ . The obtained results are shown in Table 5.

TABLE 5

| Steel symbol | Chemical component (% ratio by mass) |      |       |       |        |        |        | Number of times of punching<br>(1,000 times) |
|--------------|--------------------------------------|------|-------|-------|--------|--------|--------|----------------------------------------------|
|              | C                                    | Si   | Mn    | Al    | N      | S      | O      |                                              |
| A            | 0.0032                               | 3.25 | 0.073 | 0.008 | 0.0015 | 0.0012 | 0.0016 | 95.0                                         |
| B            | 0.0041                               | 3.88 | 0.071 | 0.002 | 0.0043 | 0.0008 | 0.0008 | 68.5                                         |
| D            | 0.0022                               | 3.38 | 0.080 | 0.006 | 0.0024 | 0.0036 | 0.0032 | 84.0                                         |
| Z            | 0.0060                               | 3.48 | 0.074 | 0.025 | 0.0080 | 0.0030 | 0.0048 | 4.5                                          |

As can be seen from Table 5, when primary recrystallization annealing is performed in a nitrogen atmosphere having a dew point of 0°C. or lower, the number of times of punching reaches 60000 or more. However, with a conventional composition, when primary recrystallization annealing causing decarburization is performed with a dew point of 60°C. by a conventional means, and when finish annealing (including purification annealing) is performed at a high temperature of 1200°C. or higher (Steel Symbol Z), the number of times of punching is several thousands. In any one of Experimental materials A to D, secondary recrystallized grains were steadily grown.

In the examples, the existence rate of fine crystal grains of 0.15 to 0.50 mm was 2 grains/cm<sup>2</sup> or more.

Then, the thus-obtained primary recrystallized sheet was coated with the annealing separator mainly composed of SiO<sub>2</sub>, and secondary recrystallization annealing was performed at an annealing temperature of 900°C. in a nitrogen atmosphere (a dew point of -10°C.) under heating from 300°C. to 800°C. at a rate of 25°C./h to obtain a grain

oriented electromagnetic steel sheet. Then, the steel sheet was coated with an organic coating mainly composed of acrylic resin and vinyl acetate, and dried by baking to obtain a product. In the examples, the Al amount of steel after final annealing was 10 to 60 ppm. Since Steel Symbol J was not decarburized, the product sheet contained substantially the same amount of C as the slab.

Table 6 also shows the magnetic properties and punching quality of the obtained products. The punching test was carried out by the same method as Example 4. Table 6 indicates that with a composition within our range, both the magnetic properties and punching quality are improved.

In the examples, the existence rate of fine crystal grains of 0.15 to 0.50 mm was 2 grains/cm<sup>2</sup> or more.

TABLE 6

| Steel symbol | Chemical component (% ratio by mass) |      |       |       |        |        |                              | Electromagnetic properties |      | Number of times of punching<br>(1,000 times) | Remarks |
|--------------|--------------------------------------|------|-------|-------|--------|--------|------------------------------|----------------------------|------|----------------------------------------------|---------|
|              | C                                    | Si   | Mn    | Al    | N      | O      | W <sub>17/50</sub><br>(w/kg) | B <sub>8</sub> (T)         |      |                                              |         |
| E            | 0.0032                               | 3.25 | 0.073 | 0.008 | 0.0015 | 0.0016 | 0.986                        | 1.92                       | 95.0 | Example                                      |         |
| F            | 0.0041                               | 3.38 | 0.151 | 0.002 | 0.0023 | 0.0008 | 1.121                        | 1.89                       | 68.5 | Example                                      |         |
| H            | 0.0033                               | 4.01 | 0.041 | 0.003 | 0.0031 | 0.0039 | 1.139                        | 1.88                       | 52.5 | Example                                      |         |
| I            | 0.0123                               | 3.38 | 0.080 | 0.006 | 0.0014 | 0.0022 | 1.536                        | 1.71                       | 14.0 | Comparative example                          |         |
| J            | 0.0048                               | 1.03 | 0.069 | 0.006 | 0.0025 | 0.0020 | 1.845                        | 1.68                       | 67.0 | Comparative example                          |         |
| L            | 0.0021                               | 3.28 | 0.075 | 0.042 | 0.0036 | 0.0011 | 1.701                        | 1.72                       | 72.5 | Comparative example                          |         |
| M            | 0.0038                               | 3.26 | 0.070 | 0.010 | 0.0072 | 0.0012 | 1.598                        | 1.69                       | 62.0 | Comparative example                          |         |

## Example 5

## First Aspect

Steel slabs containing the components shown in Table 6 (30 ppm or less each of other impurities, and without the inhibitor components) were produced by continuous casting, and heated at 1200°C. for 20 minutes. Then, each of the steel slabs was finished to a hot-rolled sheet of 2.6 mm in thickness by hot rolling. Then, each of the hot-rolled sheets was annealed (at 1000°C. for 20 seconds), and finished to a final thickness of 0.35 mm by cold rolling. Then, primary recrystallization annealing (at 900°C. for 60 seconds) was performed in a hydrogen atmosphere having a dew point of -20°C.

## Example 6

## First Aspect

55 A steel slab containing 11 ppm of C, 2.98% of Si, 0.12% of Mn, 0.012% of Al, 0.0023% of S, 0.0014% of N, 0.0010% of O, and the balance substantially composed of Fe (30 ppm or less each of other impurities, and without the inhibitor components) was produced by continuous casting. Then, the steel slab was heated at 1200°C. for 20 minutes, and then finished to a hot-rolled sheet of 2.6 mm in thickness by hot rolling. The hot-rolled sheet was annealed (at 1000°C. for 30 seconds), and then finished to a final thickness of 0.35 mm by cold rolling. Then, primary recrystallization annealing was performed (at 970°C. for 10 seconds) in a nitrogen atmosphere having a dew point of -20°C. Then, the annealing

separator mainly composed of  $\text{SiO}_2$  was coated on the primarily recrystallized sheet, and secondary recrystallization annealing was performed under a condition in which the temperature was increased from 300° C. to 800° C. at a rate of 25° C./h in a nitrogen atmosphere, and maintained at each of the temperatures shown in Table 7. After final annealing, the Al amount of steel was 50 ppm and the S amount was 15 ppm.

Then, the thus-obtained grain oriented electromagnetic steel sheets were coated with an organic coating mainly composed of an acrylic resin and an epoxy resin, and baked. Table 7 also shows the magnetic properties and punching quality of the steel sheets. Table 7 indicates that in the case of secondary recrystallization annealing within our range and the preferred range, both the magnetic properties and punching quality are improved.

In the examples, the existence rate of fine crystal grains of 0.15 to 0.50 mm was 2 grains/cm<sup>2</sup> or more.

TABLE 7

| Secondary recrystallization annealing | Electromagnetic properties | Number of times of |                        | Remarks             |
|---------------------------------------|----------------------------|--------------------|------------------------|---------------------|
| temperature (° C.)                    | W <sub>17/50</sub> (W/kg)  | B <sub>8</sub> (T) | punching (1,000 times) |                     |
| 750                                   | 2.381                      | 1.58               | 21.5                   | Comparative example |
| 775                                   | 2.375                      | 1.57               | 33.5                   | Comparative example |
| 800                                   | 1.246                      | 1.85               | 42.5                   | Example             |
| 825                                   | 1.233                      | 1.85               | 57.0                   | Example             |
| 850                                   | 1.176                      | 1.88               | 58.0                   | Example             |
| 875                                   | 1.097                      | 1.90               | 61.5                   | Example             |
| 900                                   | 1.084                      | 1.90               | 58.5                   | Example             |
| 925                                   | 1.124                      | 1.87               | 63.0                   | Example             |
| 950                                   | 1.136                      | 1.88               | 60.5                   | Example             |
| 975                                   | 1.091                      | 1.89               | 55.0                   | Example             |
| 1000                                  | 1.185                      | 1.87               | 59.0                   | Example             |
| 1025                                  | 1.511                      | 1.77               | 38.5                   | Comparative example |
| 1050                                  | 1.489                      | 1.77               | 36.0                   | Comparative example |

In the examples of the present invention, the existence rate of fine crystal grains of 0.15 to 0.50 mm was 2 grains/cm<sup>2</sup> or more.

## Example 7

## First Aspect

A steel slab containing 28 ppm of C, 3.44% of Si, 0.08% of Mn, 0.004% of Al, 0.0013% of S, 0.0022% of N, 0.0008% of O, and the balance substantially composed of Fe (30 ppm or less each of other impurities, and without the inhibitor components) was produced by continuous casting. Then, the steel slab was heated at 1200° C. for 20 minutes, and then finished to a hot-rolled sheet of 2.6 mm in thickness by hot rolling. The hot-rolled sheet was annealed (at 900° C. for 30 seconds), and then finished to a final thickness of 0.50 mm by cold rolling. Then, primary recrystallization annealing (hydrogen: 75 vol %, nitrogen: 25 vol %, 950° C.-10 seconds) was performed with the dew point being changed as shown in Table 10. Then, secondary recrystallization annealing was performed at an annealing temperature of 900° C. (hydrogen: 75 vol %, nitrogen: 25 vol %, dew point -20° C.) without the annealing separator being applied. In the secondary recrystallization annealing, the rate of heating 300° C. to 800° C. was changed as shown in Table 10. In the examples (Steel Symbols O and P), after final annealing, the Al amount of steel was 20 to 60 ppm, and the S amount was 5 to 10 ppm. In Steel Symbols Q and R, decarburization was not performed, and thus the C contents of the product sheets were substantially the same as the slabs.

Then, the thus-obtained steel sheets were coated with an organic coating mainly composed of an acrylic resin and vinyl acetate, and baked to form products. The thus-obtained products were measured with respect to the magnetic properties and punching quality. Table 10 shows the obtained results. Table 10 indicates that in the examples, both the magnetic properties and punching quality are improved.

In the examples, the existence rate of fine crystal grains of 0.15 to 0.50 mm was 2 grains/cm<sup>2</sup> or more.

vinyl acetate, and baked to form products. In the examples, after final annealing, the Al amount of steel was 20 ppm, and the S amount was 10 ppm.

Table 8 also shows the magnetic properties and punching quality of the obtained products. Table 8 indicates that in the examples, both the magnetic properties and punching quality are improved.

In the examples, the existence rate of fine crystal grains of 0.15 to 0.50 mm was 2 grains/cm<sup>2</sup> or more.

TABLE 8

| 15 | Electromagnetic properties |                           | Number of times of |                        | Remarks             |
|----|----------------------------|---------------------------|--------------------|------------------------|---------------------|
|    | Dew point (° C.)           | W <sub>17/50</sub> (W/kg) | B <sub>8</sub> (T) | punching (1,000 times) |                     |
| 20 | 60                         | 1.473                     | 1.74               | 21.5                   | Comparative example |
|    | 50                         | 1.351                     | 1.75               | 18.5                   | Comparative example |
|    | 20                         | 1.184                     | 1.88               | 24.0                   | Example             |
|    | 10                         | 1.097                     | 1.90               | 23.5                   | Example             |
|    | 0                          | 1.084                     | 1.90               | 41.5                   | Example             |
| 25 | -10                        | 1.124                     | 1.87               | 52.0                   | Example             |
|    | -20                        | 1.036                     | 1.91               | 60.5                   | Example             |
|    | <-20                       | 1.011                     | 1.92               | 61.0                   | Example             |

Example 8

## First Aspect

35 A steel slab containing each of the compositions shown in Table 9 and the balance substantially composed of Fe (30 ppm or less each of other impurities, and without the inhibitor components) was produced by continuous casting. Then, the steel slab was heated at 1200° C. for 20 minutes, and then finished to a hot-rolled sheet of 2.6 mm in thickness by hot rolling. The hot-rolled sheet was annealed (at 900° C. for 30 seconds), and then finished to a final thickness of 0.50 mm by cold rolling. Then, primary recrystallization annealing (hydrogen: 75 vol %, nitrogen: 25 vol %, 950° C.-10 seconds) was performed with the dew point being changed as shown in Table 10. Then, secondary recrystallization annealing was performed at an annealing temperature of 900° C. (hydrogen: 75 vol %, nitrogen: 25 vol %, dew point -20° C.) without the annealing separator being applied. In the secondary recrystallization annealing, the rate of heating 300° C. to 800° C. was changed as shown in Table 10. In the examples (Steel Symbols O and P), after final annealing, the Al amount of steel was 20 to 60 ppm, and the S amount was 5 to 10 ppm. In Steel Symbols Q and R, decarburization was not performed, and thus the C contents of the product sheets were substantially the same as the slabs.

Then, the thus-obtained steel sheets were coated with an organic coating mainly composed of an acrylic resin and vinyl acetate, and baked to form products. The thus-obtained products were measured with respect to the magnetic properties and punching quality. Table 10 shows the obtained results. Table 10 indicates that in the examples, both the magnetic properties and punching quality are improved.

In the examples, the existence rate of fine crystal grains of 0.15 to 0.50 mm was 2 grains/cm<sup>2</sup> or more.

TABLE 10

| Steel symbol | Dew point (° C.) | Heating rate (° C./s) | Electromagnetic properties |                    | Number of times of punching (1,000 times) | Remarks             |
|--------------|------------------|-----------------------|----------------------------|--------------------|-------------------------------------------|---------------------|
|              |                  |                       | W <sub>17/50</sub> (W/kg)  | B <sub>8</sub> (T) |                                           |                     |
| O            | <-20             | 20                    | 1.425                      | 1.912              | 63.0                                      | Example             |
| O            | <-20             | 120                   | 1.535                      | 1.733              | 49.5                                      | Comparative example |
| O            | 50               | 20                    | 1.825                      | 1.652              | 13.0                                      | Comparative example |
| O            | 50               | 120                   | 2.000                      | 1.621              | 9.5                                       | Comparative example |
| Q            | <-20             | 20                    | 1.525                      | 1.674              | 42.5                                      | Comparative example |
| Q            | <-20             | 120                   | 1.731                      | 1.658              | 31.0                                      | Comparative example |
| Q            | 50               | 20                    | 1.656                      | 1.843              | 7.5                                       | Comparative example |
| Q            | 50               | 120                   | 1.535                      | 1.682              | 8.5                                       | Comparative example |
| R            | <-20             | 20                    | 1.668                      | 1.656              | 36.0                                      | Comparative example |
| R            | <-20             | 120                   | 1.689                      | 1.643              | 43.5                                      | Comparative example |
| R            | 50               | 20                    | 1.812                      | 1.837              | 4.5                                       | Comparative example |
| R            | 50               | 120                   | 1.780                      | 1.682              | 4.0                                       | Comparative example |

Example 9

## First Aspect

A steel slab containing each of the compositions shown in Table 9 was produced by continuous casting. Then, the steel slab was heated at 1150° C. for 30 minutes, and then finished to a hot-rolled sheet of 2.6 mm in thickness by hot rolling. The hot-rolled sheet was annealed (at 950° C. for 30 seconds), and cold rolled to an intermediate thickness of 0.80 mm. After intermediate annealing at 950° C., the annealed sheet was finished to a final thickness of 0.10 mm by cold rolling. Then, primary recrystallization annealing (hydrogen atmosphere, 950° C.-20 seconds) was performed with the dew point being changed as shown in Table 11. Then, secondary recrystallization annealing was performed at an annealing temperature of 900° C. in a nitrogen atmosphere without the annealing separator being applied. In the secondary recrystallization annealing, the rate of heating 300° C. to 800° C. was changed as shown in Table 11. In the examples (Steel Symbols O and P), after final annealing, the Al amount of steel was 20 to 60 ppm, and the S amount was 5 to 15 ppm. In Steel Symbols Q and R, decarburization was not performed, and thus the C contents of the product sheets were substantially the same as the slabs.

Then, the thus-obtained steel sheets were coated with a semi-organic coating mainly composed of an acrylic resin and chromic acid type inorganic material, and baked to form products. The thus-obtained products were measured with respect to the magnetic properties and punching quality. Table 11 shows the obtained results. Table 11 indicates that the product produced under our conditions is excellent in both the magnetic properties and punching quality.

TABLE 11

| 5  | Steel symbol  | Dew point (° C.) | Heating rate (° C./s) | Electromagnetic properties |                    | Number of times of punching (1,000 times) | Remarks             |
|----|---------------|------------------|-----------------------|----------------------------|--------------------|-------------------------------------------|---------------------|
|    |               |                  |                       | W <sub>17/50</sub> (W/kg)  | B <sub>8</sub> (T) |                                           |                     |
| 10 | O             | <-20             | 20                    | 0.821                      | 1.910              | 91.0                                      | Example             |
|    | O             | <-20             | 120                   | 1.928                      | 1.741              | 69.5                                      | Comparative example |
|    | O             | 50               | 20                    | 1.196                      | 1.823              | 15.0                                      | Comparative example |
|    | O             | 50               | 120                   | 1.600                      | 1.649              | 23.0                                      | Comparative example |
|    | Q             | <-20             | 20                    | 1.240                      | 1.775              | 61.0                                      | Comparative example |
|    | Q             | <-20             | 120                   | 1.622                      | 1.667              | 32.0                                      | Comparative example |
|    | Q             | 50               | 20                    | 1.396                      | 1.805              | 19.0                                      | Comparative example |
|    | Q             | 50               | 120                   | 1.523                      | 1.709              | 18.5                                      | Comparative example |
|    | R             | <-20             | 20                    | 1.264                      | 1.823              | 53.5                                      | Comparative example |
|    | R             | <-20             | 120                   | 1.611                      | 1.655              | 40.5                                      | Comparative example |
| 20 | R             | 50               | 20                    | 1.382                      | 1.810              | 11.5                                      | Comparative example |
|    | R             | 50               | 120                   | 1.780                      | 1.611              | 9.5                                       | Comparative example |
|    | 30            |                  |                       |                            |                    |                                           |                     |
|    | Example 10    |                  |                       |                            |                    |                                           |                     |
|    | Second Aspect |                  |                       |                            |                    |                                           |                     |

A steel slab having a composition containing 0.005% of C, 3.4% of Si, 0.07% of Mn, 0.03% of Sb, and Al and N decreased to 20 ppm and 19 ppm, respectively (30 ppm or less each of other components, and without an inhibitor components) was produced by continuous casting. Then, the steel slab was heated at 1100° C. for 20 minutes, and then hot-rolled to form a hot-rolled sheet of 2.6 mm in thickness. Then, the hot-rolled sheet was annealed by soaking at 1000° C. for 60 seconds. The annealed sheet was then finished to a final thickness of 0.35 mm by cold rolling at room temperature. After hot-rolled sheet annealing, the grain diameter before final cold rolling was 130  $\mu\text{m}$ .

Then, recrystallization annealing (a dew point of -300° C.) was performed in an atmosphere containing 75 vol % of hydrogen and 25 vol % of nitrogen under the conditions shown in Table 12. After the crystal grain diameter was measured after recrystallization annealing, final annealing was performed under a condition in which the temperature was increased to 800° C. at a rate of 500° C./h in a mixed atmosphere having a dew point of -250° C. and containing 25 vol % of nitrogen and 75 vol % of hydrogen, increased from 800° C. to 860° C. at a rate of 10° C./h, and maintained at this temperature for 20 hours. In the examples, after final annealing, the Al amount of steel was 10 ppm, and the N amount was 30 ppm.

Then, the finish annealed sheet was coated with a coating solution made by mixing aluminum bichromate, an emulsion resin and ethylene glycol, and baked at 300° C. to form a product.

The thus-obtained product sheets were measured with respect to the magnetic properties, and an EI core was formed from each of the thus-obtained product sheets by punching, and measured with respect to its iron loss (W<sub>15/50</sub>) after stress relief annealing at 750° C. for 2 hours in nitrogen.

The obtained results are shown in Table 12.

For comparison, Table 12 also shows the iron loss ( $W_{15/50}$ ) measured for an EI core produced by using each of a conventional grain oriented electromagnetic steel sheet and a non-oriented electromagnetic steel sheet having the same thickness of 0.35 mm.

TABLE 12

| No. | Recrystallization annealing                      |         | W <sub>L15/50</sub> in<br>rolling direction of<br>product sheet (W/kg) | Iron loss<br>ratio $W_{C15/50}/W_{L15/50}$ (W/kg) | Iron loss<br>of EI core<br>$W_{15/50}$ (W/kg) | Remarks                  |
|-----|--------------------------------------------------|---------|------------------------------------------------------------------------|---------------------------------------------------|-----------------------------------------------|--------------------------|
|     | Temp.<br>(° C.)                                  | Time(s) | Grain diameter<br>(μm)                                                 |                                                   |                                               |                          |
| 1   | 900                                              | 30      | 35                                                                     | 0.93                                              | 1.96                                          | 1.22 Example             |
| 2   | 925                                              | 30      | 47                                                                     | 0.90                                              | 1.94                                          | 1.19 Example             |
| 3   | 950                                              | 30      | 55                                                                     | 0.89                                              | 1.93                                          | 1.17 Example             |
| 4   | 975                                              | 10      | 71                                                                     | 0.89                                              | 1.90                                          | 1.15 Example             |
| 5   | 800                                              | 3600    | 78                                                                     | 0.93                                              | 2.24                                          | 1.33 Example             |
| 6   | 840                                              | 30      | 24                                                                     | 1.64                                              | 2.28                                          | 1.99 Comparative example |
| 7   | 1000                                             | 30      | 122                                                                    | 1.55                                              | 2.00                                          | 1.97 Comparative example |
| 8   | Grain oriented<br>electromagnetic<br>steel sheet |         | 0.90                                                                   | 4.03                                              | 1.52                                          | Comparative example      |
| 9   | Non-oriented<br>electromagnetic<br>steel sheet   |         | 1.90                                                                   | 1.29                                              | 2.11                                          | Comparative example      |

As shown in Table 12, when the grain diameter after 25 recrystallization annealing is controlled in the range of 30 to 80 μm, a product can be obtained, in which the iron loss ( $W_{L15/50}$ ) in the rolling direction is 1.40 W/kg or less, and the iron loss ( $W_{C15/50}$ ) in the direction perpendicular to the rolling direction is 2.6 times or less as large as that ( $W_{L15/50}$ ) in the rolling direction. It is thus found that a good iron loss can be obtained in application to the EI core.

In the examples, the existence rate of fine crystal grains of 0.15 to 0.50 mm is 3 grains/cm<sup>2</sup> or more.

#### Example 11

#### Second Aspect

A steel slab having a composition containing 0.023% of C, 3.3% of Si, 0.12% of Mn, and Al and N decreased to 40 ppm and 14 ppm, respectively (30 ppm or less each of other components, and without an inhibitor components) was produced by continuous casting. Then, the steel slab was heated at 1200° C. for 20 minutes, and then hot-rolled to 40 form a hot-rolled sheet of 2.2 mm in thickness. Then, the hot-rolled sheet was annealed at 1100° C. for 20 seconds. The annealed sheet was then finished to a final thickness of 0.35 mm by cold rolling at 240° C. under a condition in 50 which aging was performed at 200° C. for 5 hours when the thickness was 0.90 mm in the course of rolling. The grain diameter before final cold rolling was 280 μm.

Then, recrystallization annealing including decarburization was performed in an atmosphere containing 75 vol % of hydrogen and 25 vol % of nitrogen and having a dew point of 50° C. under the conditions shown in Table 13. After the 30 crystal grain diameter was measured after recrystallization annealing, colloidal silica ( $SiO_2$ ) was coated as the annealing separator, and then final annealing (an annealing atmosphere containing 75 vol % of hydrogen and 25 vol % of nitrogen, and having a dew point of -20° C.) was performed 35 under a condition in which the temperature was increased from room temperature to 900° C. at a rate of 300° C./h, and maintained at this temperature for 50 hours. In the examples, after final annealing, the C amount of steel was 10 ppm, the Al amount of steel was 10 ppm, and the N amount of steel 40 was 15 ppm.

Then, the finish annealed sheet was coated with a coating 45 solution made by mixing aluminum bichromate, an emulsion resin and ethylene glycol, and baked at 300° C. to form a product.

The thus-obtained product sheets were measured with respect to the magnetic properties, and an EI core formed 50 from each of the thus-obtained product sheets by punching, was measured with respect to its iron loss ( $W_{15/50}$ ) after stress relief annealing (at 750° C. for 2 hours in nitrogen). The obtained results are shown in Table 13.

TABLE 13

| No. | Recrystallization annealing |         | W <sub>L15/50</sub> in<br>rolling direction<br>of product<br>sheet (W/kg) | Iron loss<br>ratio<br>$W_{C15/50}/W_{L15/50}$ (W/kg) | Direction<br>perpendicular to<br>rolling direction<br>$B_{L50}$ (T) | Direction<br>perpendicular to<br>rolling direction<br>$B_{C50}$ (T) | Iron loss of<br>EI core<br>$W_{15/50}$ (W/kg) | Remarks                  |
|-----|-----------------------------|---------|---------------------------------------------------------------------------|------------------------------------------------------|---------------------------------------------------------------------|---------------------------------------------------------------------|-----------------------------------------------|--------------------------|
|     | Temp.<br>(° C.)             | Time(s) | Grain diameter<br>(μm)                                                    |                                                      |                                                                     |                                                                     |                                               |                          |
| 1   | 850                         | 60      | 32                                                                        | 1.05                                                 | 1.36                                                                | 1.95                                                                | 1.85                                          | 1.12 Example             |
| 2   | 875                         | 60      | 45                                                                        | 1.03                                                 | 1.33                                                                | 1.95                                                                | 1.87                                          | 1.08 Example             |
| 3   | 900                         | 60      | 57                                                                        | 1.04                                                 | 1.24                                                                | 1.92                                                                | 1.90                                          | 1.06 Example             |
| 4   | 925                         | 30      | 70                                                                        | 1.08                                                 | 1.20                                                                | 1.90                                                                | 1.91                                          | 1.10 Example             |
| 5   | 800                         | 3600    | 75                                                                        | 1.15                                                 | 1.44                                                                | 1.94                                                                | 1.78                                          | 1.25 Example             |
| 6   | 800                         | 30      | 20                                                                        | 1.85                                                 | 1.50                                                                | 1.75                                                                | 1.63                                          | 1.97 Comparative example |
| 7   | 1000                        | 30      | 111                                                                       | 1.99                                                 | 1.44                                                                | 1.73                                                                | 1.60                                          | 2.03 Comparative example |

As shown in Table 13, when the grain diameter after recrystallization annealing is controlled in the range of 30 to 80  $\mu\text{m}$ , a product can be obtained, in which the iron loss ( $W_{L15/50}$ ) in the rolling direction is 1.40 W/kg or less, and the iron loss ( $W_{C15/50}$ ) in the direction perpendicular to the rolling direction is 2.6 times or less as large as that ( $W_{L15/50}$ ) in the rolling direction. It is thus found that a good iron loss can be obtained in application to the EI core.

In the examples, the existence rate of fine crystal grains of 0.15 to 0.50 mm is 3 grains/cm<sup>2</sup> or more.

### Example 12

#### Second Aspect

Steel slabs containing the components shown in Table 14 (30 ppm or less each of other impurities, and without the inhibitor components) were heated to 1160° C., and hot-rolled to form hot-rolled sheets of 2.6 mm in thickness. Then, each of the hot-rolled sheets was annealed by soaking at 1000° C. for 30 seconds. The crystal grain diameter before the start of cold rolling was 30 to 60  $\mu\text{m}$ . Then, each annealed sheet was finished to a final thickness of 0.30 mm by cold rolling. Then, primary recrystallization annealing was performed by soaking at 980° C. for 20 seconds in an atmosphere containing 50 vol % of hydrogen and 50 vol % of nitrogen, and having a dew point of -30° C. After the grain diameter after recrystallization annealing was measured, final annealing was performed in a nitrogen atmosphere having a dew point of -40° C. under a condition in which the temperature was increased to 850° C. at a rate of 10° C./h, and maintained at this temperature for 75 hours without the annealing separator being applied. In the examples, after final annealing, the Al amount of steel was 5 to 30 ppm, and the N amount was 15 to 50 ppm.

Then, the steel sheet was coated with a coating solution made by mixing aluminum phosphate, potassium bichromate and boric acid, and baked at 300° C. to obtain a product.

The thus-obtained product sheet was measured with respect to the magnetic properties, and an EI core produced by using each of the product sheets was measured with respect to its iron loss ( $W_{15/50}$ ) after stress relief annealing (at 750° C. for 2 hours in nitrogen). The obtained results are shown in Table 14.

Table 14 indicates that by using a slab of a component system satisfying 0.003 to 0.08% of C, 2.0% to 8.0% of Si, 100 ppm or less of Al, and 30 ppm or less of N, a product can be obtained, in which the iron loss ( $W_{L15/50}$ ) in the rolling direction is 1.40 W/kg or less, and the iron loss ( $W_{C15/50}$ ) in the direction perpendicular to the rolling direction is 2.6 times or less as large as that ( $W_{L15/50}$ ) in the rolling direction.

In the examples, the existence rate of fine crystal grains of 0.15 to 0.50 mm was 3 grains/cm<sup>2</sup> or more.

### Example 13

#### Third Aspect

A steel slab containing 0.002% of C, 3.5% of Si, 0.05% of Mn, 0.02% of Sb, Al and N decreased to 40 ppm and 9 ppm, respectively, and 20 ppm or less each of other impurities (without the inhibitor components) was produced by continuous casting, and heated at 1100° C. for 20 minutes. Then, the steel slab was hot-rolled to form a hot-rolled sheet of 2.6 mm in thickness. Then, the hot-rolled sheet was annealed by soaking at 1000° C. for 60 seconds. Then, first cold rolling was performed at room temperature to obtain an intermediate thickness of 1.60 mm, and intermediate annealing was performed by soaking at 850° C. for 10 seconds. The crystal grain diameter after intermediate annealing was 70  $\mu\text{m}$ .

Then, the annealed sheet was finished to a final thickness of 0.20 mm by second cold rolling at room temperature under a condition in which aging was performed at 200° C. for 5 hours when the thickness was 0.90 mm in the course of cold rolling. Then, recrystallization annealing was performed in a mixed atmosphere containing 75 vol % of hydrogen and 25 vol % of nitrogen (a dew point of -50° C.) under the conditions shown in Table 15. After the grain diameter after recrystallization annealing was measured, final annealing was performed under a condition in which the temperature was increased to 800° C. at a rate of 50° C./h in an atmosphere having a dew point of -50° C. and containing 25 vol % of nitrogen and 75 vol % of hydrogen, increased from 800° C. to 830° C. at a rate of 10° C./h, and maintained at this temperature for 50 hours without the

TABLE 14

| No. | Chemical composition (mass %, ppm) |      |      |      |      |      |      |      |    |      | Recrystallized grain diameter | $W_{L15/50}$ in rolling direction | Iron loss ratio |              | EI core | Remarks             |         |
|-----|------------------------------------|------|------|------|------|------|------|------|----|------|-------------------------------|-----------------------------------|-----------------|--------------|---------|---------------------|---------|
|     | C                                  | Si   | Mn   | Ni   | Sn   | Sb   | Cu   | P    | Cr | Al   |                               |                                   | (W/kg)          | $W_{L15/50}$ | (W/kg)  |                     |         |
| 1   | 15                                 | 3.32 | 0.12 | tr   | tr   | Tr   | tr   | tr   | tr | 30   | 20                            | 56                                | 0.85            | 2.04         | 1.20    | Example             |         |
| 2   | 14                                 | 3.40 | 0.05 | 0.30 | tr   | tr   | tr   | tr   | tr | 17   | 13                            | 65                                | 0.80            | 1.95         | 1.15    | Example             |         |
| 3   | 20                                 | 3.45 | 0.22 | tr   | 0.14 | tr   | tr   | tr   | tr | 50   | 25                            | 44                                | 0.85            | 1.77         | 1.10    | Example             |         |
| 4   | 24                                 | 3.22 | 0.13 | tr   | tr   | 0.03 | tr   | tr   | tr | 66   | 12                            | 63                                | 0.83            | 1.75         | 1.07    | Example             |         |
| 5   | 22                                 | 3.32 | 0.08 | tr   | tr   | tr   | 0.15 | tr   | tr | 25   | 6                             | 67                                | 0.81            | 1.84         | 1.10    | Example             |         |
| 6   | 16                                 | 3.45 | 0.10 | tr   | tr   | tr   | tr   | 0.08 | tr | 30   | 15                            | 48                                | 0.83            | 1.95         | 1.17    | Example             |         |
| 7   | 20                                 | 3.40 | 0.37 | tr   | tr   | tr   | tr   | tr   | tr | 0.50 | 35                            | 10                                | 50              | 0.80         | 1.80    | 1.08                | Example |
| 8   | 13                                 | 3.37 | 0.16 | tr   | tr   | tr   | tr   | tr   | tr | 250  | 20                            | 13                                | 1.88            | 1.56         | 2.23    | Comparative example |         |
| 9   | 16                                 | 3.41 | 0.20 | tr   | tr   | tr   | tr   | tr   | tr | 50   | 85                            | 19                                | 2.10            | 1.44         | 2.33    | Comparative example |         |

annealing separator being applied. In the examples, after final annealing, the Al amount of steel was 20 ppm, and the N amount was 20 ppm.

Then, the steel sheet was coated with a coating solution made by mixing aluminum bichromate, an emulsion resin and ethylene glycol, and baked at 300° C. to obtain a product.

The thus-obtained product sheet was measured with respect to the average grain diameter of the secondary recrystallized grains on the surface of the steel sheet except fine grains of 1 mm or less.

Also, the existence rate of fine crystal grains having a grain diameter of 0.15 mm to 1.00 mm in the secondary recrystallized grains was determined by measuring the number of the fine crystal grains in a 3-cm square region of the surface of the steel sheet.

Furthermore, crystal orientation of the product sheet was measured in a region of 30×280 mm by X-ray diffraction to measure the rate (area fraction) of crystal grains having Goss orientation allowing 20° of the deviation angle from ideal {110}<001> orientation (area fraction of Goss orientation grains).

Furthermore, a high-frequency iron loss (frequency: 400 Hz, 1000 Hz), was measured at a frequency of each of 400 Hz and 1000 Hz.

The obtained results are shown in Table 15.

For comparison, Table 15 also shows the results of the same measurement conducted for a grain oriented electromagnetic steel sheet and a non-oriented electromagnetic steel sheet having the same thickness of 0.20 mm.

respectively, (30 ppm or less each of other impurities, and without the inhibitor components) was produced by continuous casting, and heated at 1200° C. for 20 minutes. Then, the steel slab was hot-rolled to form a hot-rolled sheet of 2.2 mm in thickness, and the hot-rolled sheet was annealed by soaking at 900° C. for 30 seconds. Then, first cold rolling was performed at room temperature to finish the sheet to a thickness of 0.30 mm, and intermediate annealing was performed under the conditions shown in Table 16. Then, the annealed sheet was finished to a final thickness of 0.10 mm by second cold rolling at room temperature.

Then, recrystallization annealing was performed by soaking at 900° C. for 10 seconds in an atmosphere containing 75 vol % of hydrogen and 25 vol % of nitrogen and having a dew point of -500° C. After the grain diameter after recrystallization annealing was measured, colloidal silica was applied as the annealing separator, and then final annealing was performed under a condition in which the temperature was increased from room temperature to 900° C. at a rate of 30° C./h, and maintained at this temperature for 50 hours (atmosphere, hydrogen: 75 vol %, nitrogen: 25 vol %, dew point: -30° C.). In the examples, after final annealing, the Al amount of steel was 10 ppm, and the N amount was 20 ppm.

Then, the steel sheet was coated with a coating solution made by mixing aluminum bichromate, an emulsion resin and ethylene glycol, and baked at 300° C. to obtain a product.

TABLE 15

| No. | Recrystallization annealing                |         | Iron loss of product sheet |                            | product sheet (mm)          | Rate of fine grains of product sheet (/cm <sup>2</sup> ) | Area ratio of Goss orientation grains of product sheet (%) | Remarks             |
|-----|--------------------------------------------|---------|----------------------------|----------------------------|-----------------------------|----------------------------------------------------------|------------------------------------------------------------|---------------------|
|     | Temp. (° C.)                               | Time(s) | Grain diameter (μm)        | W <sub>10/400</sub> (W/kg) | W <sub>10/1000</sub> (W/kg) |                                                          |                                                            |                     |
| 1   | 880                                        | 30      | 33                         | 6.7                        | 28.0                        | 37                                                       | 219                                                        | 94                  |
| 2   | 915                                        | 30      | 44                         | 6.1                        | 27.1                        | 45                                                       | 188                                                        | 99                  |
| 3   | 940                                        | 30      | 55                         | 6.5                        | 28.6                        | 34                                                       | 198                                                        | 95                  |
| 4   | 965                                        | 10      | 70                         | 6.8                        | 29.0                        | 25                                                       | 156                                                        | 95                  |
| 5   | 800                                        | 3600    | 77                         | 7.3                        | 29.7                        | 18                                                       | 133                                                        | 88                  |
| 6   | 800                                        | 30      | 23                         | 8.9                        | 33.7                        | 5                                                        | 28                                                         | 70                  |
| 7   | 1000                                       | 30      | 120                        | 9.4                        | 34.1                        | 3                                                        | 197                                                        | 66                  |
| 8   | Grain oriented electromagnetic steel sheet |         | 8.5                        | 34.0                       | 22                          | 0.2                                                      | 98                                                         | Comparative example |
| 9   | Non-oriented electromagnetic steel sheet   |         | 11.0                       | 39.8                       | 0.10                        | —                                                        | 5                                                          | Comparative example |

Table 15 indicates that in any of the examples, a high-frequency iron loss superior to a conventional grain oriented electromagnetic steel sheet is obtained.

In the examples, the existence rate of fine crystal grains of 0.15 to 0.50 mm was 2 grains/cm<sup>2</sup> or more.

#### Example 14

##### Third Aspect

A steel slab containing 0.003% of C, 3.6% of Si, 0.12% of Mn, and Al and N decreased to 30 ppm and 10 ppm,

The thus-obtained product sheet was measured with respect to the average grain diameter of the secondary recrystallized grains, the existence rate of fine crystal grains, the area ratio of Goss orientation grains, and the high-frequency iron loss at each of the frequencies in the same manner as Example 13.

The obtained results are shown in Table 16.

For comparison, Table 16 also shows the results of the same measurement conducted for a non-oriented electromagnetic steel sheet having the same thickness of 0.10 mm and a composition containing 6.5% of Si.

TABLE 16

| No. | Intermediate annealing                           |         | Grain diameter after recrystallization annealing (μm) | Iron loss of product sheet |                            | Average grain diameter of product sheet (mm) | Rate of fine grains of product sheet (/cm <sup>2</sup> ) | Area ratio of Goss orientation grains of product sheet (%) | Remarks                |
|-----|--------------------------------------------------|---------|-------------------------------------------------------|----------------------------|----------------------------|----------------------------------------------|----------------------------------------------------------|------------------------------------------------------------|------------------------|
|     | Temp. (° C.)                                     | Time(s) |                                                       | Grain diameter (μm)        | W <sub>10/400</sub> (W/kg) | W <sub>10/1000</sub> (W/kg)                  |                                                          |                                                            |                        |
| 1   | 850                                              | 30      | 30                                                    | 46                         | 4.7                        | 18.0                                         | 23                                                       | 202                                                        | 83 Example             |
| 2   | 900                                              | 30      | 43                                                    | 49                         | 4.1                        | 17.0                                         | 25                                                       | 105                                                        | 91 Example             |
| 3   | 925                                              | 30      | 51                                                    | 52                         | 5.0                        | 18.6                                         | 18                                                       | 133                                                        | 80 Example             |
| 4   | 950                                              | 10      | 66                                                    | 43                         | 5.2                        | 18.8                                         | 15                                                       | 175                                                        | 73 Example             |
| 5   | 800                                              | 3600    | 73                                                    | 35                         | 5.3                        | 18.7                                         | 13                                                       | 863                                                        | 81 Example             |
| 6   | 1000                                             | 30      | 330                                                   | 28                         | 9.4                        | 24.3                                         | 17                                                       | 76                                                         | 26 Comparative example |
| 7   | (Electromagnetic steel sheet containing 6.5% Si) |         | —                                                     | 5.7                        | 19.0                       | 0.25                                         | —                                                        | 4                                                          | Comparative example    |

Table 16 indicates that in any of the examples, a high-frequency iron loss superior to the conventional non-oriented electromagnetic steel sheet containing 6.5% of Si is obtained.

In the examples, the existence rate of fine crystal grains of 0.15 to 0.50 mm was 2 grains/cm<sup>2</sup> or more.

#### Example 15

##### Third aspect

Steel slabs having the compositions shown in Table 17 30 ppm or less each of other components, and without the inhibitor components) were produced by continuous casting, and heated to 1160° C. Then, each of the steel slabs was hot-rolled to form a hot-rolled sheet of 1.6 mm in thickness, and the hot-rolled sheet was annealed by soaking at 850° C. for 30 seconds. Then, cold rolling was performed to finish the sheet to a final thickness of 0.23 mm. Before cold rolling, the grain diameter was 40 to 60 μm.

Then, recrystallization annealing was performed by soaking at 950° C. for 10 seconds in an atmosphere containing 50 vol % of hydrogen and 50 vol % of nitrogen and having

a dew point of -30° C. After the grain diameter after recrystallization annealing was measured, final annealing was performed under a condition in which the temperature was increased to 850° C. at a rate of 10° C./h, and maintained at this temperature for 75 hours in a nitrogen atmosphere having a dew point of -4 0° C., without the annealing separator being applied. In the examples, after final annealing, the Al amount of steel was 5 to 30 ppm, and the N amount was 20 to 40 ppm.

Then, the steel sheet was coated with a coating solution made by mixing aluminum phosphate, potassium bichromate, and boric acid, and baked at 300° C. to obtain a product.

The thus-obtained product sheet was measured with respect to the average grain diameter of the secondary recrystallized grains, the existence rate of fine crystal grains, the area ratio of Goss orientation grains, and the high-frequency iron loss at a frequency of 1000 Hz in the same manner as Example 13.

The obtained results are shown in Table 18.

For comparison, Table 18 also shows the results of the same measurement conducted for a grain oriented electromagnetic steel sheet having the same thickness of 0.23 mm.

TABLE 17

| No. | Chemical composition (mass %, ppm)           |      |      |      |      |      |      |      |      |     |    |
|-----|----------------------------------------------|------|------|------|------|------|------|------|------|-----|----|
|     | C                                            | Si   | Mn   | Ni   | Sn   | Sb   | Cu   | P    | Cr   | Al  | N  |
| 1   | 25                                           | 3.52 | 0.10 | tr   | tr   | tr   | tr   | tr   | tr   | 20  | 21 |
| 2   | 24                                           | 3.50 | 0.05 | 0.50 | tr   | tr   | tr   | tr   | tr   | 20  | 19 |
| 3   | 30                                           | 3.53 | 0.20 | tr   | 0.04 | tr   | tr   | tr   | tr   | 50  | 22 |
| 4   | 33                                           | 3.62 | 0.15 | tr   | tr   | 0.04 | tr   | tr   | tr   | 60  | 22 |
| 5   | 25                                           | 3.52 | 0.08 | tr   | tr   | tr   | 0.10 | tr   | tr   | 10  | 15 |
| 6   | 13                                           | 3.51 | 0.12 | tr   | tr   | tr   | tr   | 0.04 | tr   | 30  | 12 |
| 7   | 41                                           | 3.30 | 0.07 | tr   | tr   | tr   | tr   | tr   | 0.30 | 30  | 10 |
| 8   | 23                                           | 3.48 | 0.06 | tr   | tr   | tr   | tr   | tr   | tr   | 240 | 20 |
| 9   | 15                                           | 3.49 | 0.20 | tr   | tr   | tr   | tr   | tr   | tr   | 50  | 80 |
| 10  | (Grain oriented electromagnetic steel sheet) |      |      |      |      |      |      |      |      |     |    |

TABLE 18

| No. | Grain diameter after recrystallization annealing (μm) | Iron loss of product sheet W <sub>10/1000</sub> (W/kg) | Average grain diameter of secondary recrystallized grains (mm) | Rate of fine grains (/cm <sup>2</sup> ) | Area fraction of Goss orientation grains (%) | Remarks |
|-----|-------------------------------------------------------|--------------------------------------------------------|----------------------------------------------------------------|-----------------------------------------|----------------------------------------------|---------|
|     |                                                       |                                                        |                                                                |                                         |                                              |         |
| 1   | 45                                                    | 32.0                                                   | 45                                                             | 98                                      | 87                                           | Example |
| 2   | 45                                                    | 30.5                                                   | 55                                                             | 66                                      | 89                                           | Example |
| 3   | 44                                                    | 31.0                                                   | 23                                                             | 115                                     | 90                                           | Example |
| 4   | 43                                                    | 30.6                                                   | 46                                                             | 55                                      | 91                                           | Example |

TABLE 18-continued

| No. | Grain diameter after recrystallization annealing (μm) | Iron loss of product sheet W <sub>10/1000</sub> (W/kg) | Average grain diameter of secondary recrystallized grains (mm) | Rate of fine grains (/cm <sup>2</sup> ) | Area fraction of Goss orientation grains (%) | Remarks             |
|-----|-------------------------------------------------------|--------------------------------------------------------|----------------------------------------------------------------|-----------------------------------------|----------------------------------------------|---------------------|
| 5   | 45                                                    | 31.2                                                   | 44                                                             | 68                                      | 90                                           | Example             |
| 6   | 49                                                    | 31.2                                                   | 33                                                             | 102                                     | 90                                           | Example             |
| 7   | 50                                                    | 30.5                                                   | 27                                                             | 99                                      | 85                                           | Example             |
| 8   | 12                                                    | 43.5                                                   | 5                                                              | 150                                     | 20                                           | Comparative example |
| 9   | 20                                                    | 36.8                                                   | 5                                                              | 221                                     | 35                                           | Comparative example |
| 10  | Grain oriented electromagnetic steel sheet            | 35.2                                                   | 25                                                             | 0.1                                     | 95                                           | Comparative example |

Table 18 indicates that in any of the examples, a high-frequency iron loss superior to the conventional grain oriented electromagnetic steel sheet is obtained.

In the examples, the existence rate of fine crystal grains of 0.15 to 0.50 mm was 2 grains/cm<sup>2</sup> or more.

#### INDUSTRIAL APPLICABILITY

An excellent grain oriented electromagnetic steel sheet not having a hard coating such as a forsterite undercoating or the like on its surface can be remarkably economically produced. The grain oriented electromagnetic steel sheet is excellent in punching quality and a like, and can thus significantly economize the process for producing, for example, an EI core.

Also, a grain oriented electromagnetic steel sheet having excellent properties such as good punching quality, a low iron loss and/or high-frequency iron loss, magnetic properties with low anisotropy, etc. can be stably obtained by using a raw material containing high-purity components without an inhibitor.

Particularly, in the first aspect, a grain oriented electromagnetic steel sheet having the properties of excellent punching quality and iron loss can be stably obtained, in the second aspect, a grain oriented electromagnetic steel sheet having the properties of excellent punching quality and magnetic properties, and low anisotropy in the magnetic properties can be stably obtained, and in the third aspect, a grain oriented electromagnetic steel sheet having the properties of an excellent high-frequency iron loss can be stably obtained.

Furthermore, a raw material does not contain inhibitor components, and thus a slab need not be heated at high temperature, and subjected to decarburization annealing and high-temperature purification annealing, thereby causing the great advantage that mass production can be realized at low cost.

In the first and second aspects, the use of an EI core as a core is mainly described. However, needless to say, application of the steel sheet is not limited to the EI core, and the steel sheet can be used to all applications of grain oriented electromagnetic steel sheets in which processability is regarded as important.

The invention claimed is:

1. A method of producing a grain oriented electromagnetic steel sheet having excellent magnetic properties without an undercoating mainly composed of forsterite comprising:

hot-rolling a steel slab having a composition that is substantially free of inhibitors and contains, by % by

mass, 0.08% or less of C, 1.0 to 8.0% of Si, and 0.005 to 3.0% of Mn, and Al and N each decreased to 0.020% or less and 50 ppm or less, respectively;

annealing the hot-rolled sheet according to demand; cold-rolling the sheet once, or twice or more with intermediate annealing performed therebetween; recrystallization annealing the cold-rolled sheet; and final batch annealing the sheet at a temperature of 1000°

C. or lower in a low oxidizing or non-oxidizing atmosphere having a dew point of 40° C. or lower after an annealing separator not containing MgO is coated according to demand.

2. The method of according to claim 1, wherein the steel slab further contains, by % by mass, at least one selected from 0.005 to 1.50% of Ni, 0.01 to 1.50% of Sn, 0.005 to 0.50% of Sb, 0.01 to 1.50% of Cu, 0.005 to 0.50% of P, 0.005 to 0.50% of Mo, and 0.01 to 1.50% of Cr.

3. The method according to claim 1, wherein the steel slab comprises a composition containing 2.0% by mass or more of Si.

4. The method according to claim 1, wherein the steel slab comprises a composition in which Al is decreased to 100 ppm or less.

5. The method according to claim 1, wherein the final annealing is performed in an atmosphere containing nitrogen.

6. The method according to claim 1, wherein the slab heating temperature before hot rolling is 1300° C. or lower.

7. The method according to claim 1, wherein the recrystallization annealing is performed in a low-oxidizing or non-oxidizing atmosphere having a dew point of 40° C. or lower.

8. The method according to claim 1, wherein the grain diameter after recrystallization annealing is 30 to 80 μm, and the final annealing is performed at a temperature of 975° C. or lower.

9. The method according to claim 8, wherein, in the cold rolling or rollings, the grain diameter before final cold rolling is less than 150 μm.

10. The method according to claim 8, wherein, in the cold rolling or rollings, the grain diameter before final cold rolling is 150 μm or more.

11. The method according to claim 1, wherein the highest heating temperature of the final annealing is 800° C. or higher, and the rate of heating from 300° C. to 800° C. in the final annealing is 5 to 100° C./h.

12. The method according to claim 11, wherein the steel slab contains, by % by mass, 0.006% or less of C, 2.5 to 4.5% of Si, 0.50% or less of Mn, O suppressed to 50 ppm or less, and the balance substantially composed of Fe and

**53**

inevitable impurities, and the atmosphere of the recrystallization annealing has a dew point of 0° C. or lower.

**13.** The method according to claim 1, wherein the steel sheet is coated with an insulating coating after the final annealing, and then baked.

**14.** The method according to claim 1, wherein the final annealing causes secondary recrystallized grains of the steel sheet to contain fine crystal grains passing through the sheet in the thickness direction having a grain diameter of about 0.15 mm to 0.50 mm at a rate of 2 grains/cm<sup>2</sup> or more.

**15.** The method according to claim 1, wherein the final batch annealing causes fine crystal grains having a grain

**54**

diameter of about 0.15 mm to 0.50 mm to be scattered in secondary recrystallized coarse grains that are as large as several cm.

**16.** The method according to claim 15, wherein the fine crystal grains have a grain diameter of about 0.15 mm to 0.50 mm at a rate of 2 grains/cm<sup>2</sup> or more and passes through the sheet in the thickness direction.

**17.** The method according to claim 1, wherein the steel slab contains 0.50% or less of Mn.

\* \* \* \* \*

UNITED STATES PATENT AND TRADEMARK OFFICE  
**CERTIFICATE OF CORRECTION**

PATENT NO. : 7,371,291 B2  
APPLICATION NO. : 11/145705  
DATED : May 13, 2008  
INVENTOR(S) : Hayakawa et al.

Page 1 of 1

It is certified that error appears in the above-identified patent and that said Letters Patent is hereby corrected as shown below:

In Column 7

At line 36, please change "(B<sub>50</sub>)" to -- (B<sub>c50</sub>) --.

In Column 23

At line 24, please change "100020" to -- 1000 --.

In Column 42

At line 45, please change "-300" to -- 30 --; at line 51, please change "500" to -- -50 --; and at line 52, please change "-250" to -- -25 --.

In Column 48

At line 16, please change "-500" to -- -50 --.

In Column 50

At table 16, at the subheading "Rate of fine grains of product sheet", at No. 5, please change "863" to -- 83 --.

Signed and Sealed this

Tenth Day of March, 2009



JOHN DOLL  
*Acting Director of the United States Patent and Trademark Office*

UNITED STATES PATENT AND TRADEMARK OFFICE  
**CERTIFICATE OF CORRECTION**

PATENT NO. : 7,371,291 B2  
APPLICATION NO. : 11/145705  
DATED : May 13, 2008  
INVENTOR(S) : Hayakawa et al.

Page 1 of 1

It is certified that error appears in the above-identified patent and that said Letters Patent is hereby corrected as shown below:

In Column 7

At line 36, please change "(B<sub>50</sub>)" to -- (B<sub>c50</sub>) --.

In Column 23

At line 24, please change "100020" to -- 1000 --.

In Column 42

At line 45, please change "-300" to -- 30°C --; at line 51, please change "500" to -- -50 --; and at line 52, please change "-250" to -- -25 --.

In Column 48

At line 16, please change "-500" to -- -50 --.

In Column 50

At table 16, at the subheading "Rate of fine grains of product sheet", at No. 5, please change "863" to -- 83 --.

This certificate supersedes the Certificate of Correction issued March 10, 2009.

Signed and Sealed this

Twenty-sixth Day of May, 2009



JOHN DOLL  
*Acting Director of the United States Patent and Trademark Office*

UNITED STATES PATENT AND TRADEMARK OFFICE  
**CERTIFICATE OF CORRECTION**

PATENT NO. : 7,371,291 B2  
APPLICATION NO. : 11/145705  
DATED : May 13, 2008  
INVENTOR(S) : Hayakawa et al.

Page 1 of 1

It is certified that error appears in the above-identified patent and that said Letters Patent is hereby corrected as shown below:

In Column 7

At line 36, please change "(B<sub>50</sub>)" to -- (B<sub>c50</sub>) --.

In Column 23

At line 24, please change "100020" to -- 1000 --.

In Column 42

At line 45, please change "-300°C" to -- 30°C --; at line 51, please change "500" to -- -50 --; and at line 52, please change "-250" to -- -25 --.

In Column 48

At line 16, please change "-500" to -- -50 --.

In Column 50

At table 16, at the subheading "Rate of fine grains of product sheet", at No. 5, please change "863" to -- 83 --.

This certificate supersedes the Certificates of Correction issued March 10, 2009 and May 26, 2009.

Signed and Sealed this

Thirtieth Day of June, 2009



JOHN DOLL  
*Acting Director of the United States Patent and Trademark Office*

UNITED STATES PATENT AND TRADEMARK OFFICE  
**CERTIFICATE OF CORRECTION**

PATENT NO. : 7,371,291 B2  
APPLICATION NO. : 11/145705  
DATED : May 13, 2008  
INVENTOR(S) : Hayakawa et al.

Page 1 of 1

It is certified that error appears in the above-identified patent and that said Letters Patent is hereby corrected as shown below:

In Column 7

At line 36, please change "(B<sub>50</sub>)" to -- (B<sub>c50</sub>) --.

In Column 23

At line 24, please change "100020" to -- 1000 --.

In Column 42

At line 45, please change "-300°C" to -- -30°C --; at line 51, please change "500" to -- -50 --; and at line 52, please change "-250" to -- -25 --.

In Column 48

At line 16, please change "-500" to -- -50 --.

In Column 50

At table 16, at the subheading "Rate of fine grains of product sheet", at No. 5, please change "863" to -- 83 --.

This certificate supersedes all previously issued Certificates of Correction.

Signed and Sealed this

Eighteenth Day of August, 2009



David J. Kappos  
Director of the United States Patent and Trademark Office